

Dec. 22, 1964

F. S. ROSTLER  
METHODS FOR IMPROVEMENT OF ASPHALTS AND OIL  
EMULSIONS USEFUL THEREIN

3,162,101

Filed April 19, 1963

5 Sheets-Sheet 1



INVENTOR.

*Fritz S. Rostler*

BY *Philip Lubkow*

ATTORNEY.

Dec. 22, 1964

F. S. ROSTLER

3,162,101

METHODS FOR IMPROVEMENT OF ASPHALTS AND OIL  
EMULSIONS USEFUL THEREIN

Filed April 19, 1963

5 Sheets-Sheet 2

227.2



% AVERAGE ABRAISION LOSS (PELLET METHOD)

INVENTOR

*Fritz S. Rostler*

BY *Philip Subkow*

ATTORNEY

Dec. 22, 1964

F. S. ROSTLER

METHODS FOR IMPROVEMENT OF ASPHALTS AND OIL  
EMULSIONS USEFUL THEREIN

3,162,101

Filed April 19, 1963

5 Sheets-Sheet 3

FIG. 3



INVENTOR.

*Fritz S. Rostler*

BY *Philip Lubkin*

ATTORNEY.

Dec. 22, 1964

F. S. ROSTLER

3,162,101

METHODS FOR IMPROVEMENT OF ASPHALTS AND OIL  
EMULSIONS USEFUL THEREIN

Filed April 19, 1963

5 Sheets-Sheet 4



INVENTOR.  
FRITZ S. ROSTLER

BY

Philip Laskow

ATTORNEY

Dec. 22, 1964

F. S. ROSTLER

3,162,101

METHODS FOR IMPROVEMENT OF ASPHALTS AND OIL  
EMULSIONS USEFUL THEREIN

Filed April 19, 1963

5 Sheets-Sheet 5

Fritz S.



CURVE

A 48 PEN. ASPHALT WEATHERED 14 DAYS

B 48 PEN. ASPHALT UNWEATHERED

C 48 PEN. ASPHALT TREATED WITH MALTENES  
EMULSION AND WEATHERED 14 DAYS

D 200-300 PEN. ASPHALT UNWEATHERED

E 48 PEN. ASPHALT TREATED WITH MALTENES  
IN KEROSENE AND WEATHERED 14 DAYS.

Fritz S. ROSTLER  
INVENTOR.

BY *Philip Lutkow*

ATTORNEY.

# United States Patent Office

3,162,101

Patented Dec. 22, 1964

1

3,162,101

METHODS FOR IMPROVEMENT OF ASPHALTS  
AND OIL EMULSIONS USEFUL THEREIN  
Fritz S. Rostler, Bakersfield, Calif., assignor, by mesne  
assignments, to Witco Chemical Company, Inc., New  
York, N.Y., a corporation of Delaware

Filed Apr. 19, 1963, Ser. No. 274,193  
47 Claims. (Cl. 94—23)

This invention relates to methods for improving the durability of asphalts, both weathered and unweathered, by adjusting the components of the asphalt other than the asphaltenes content, to provide a favorable balance of the concentrations of these several components other than asphaltenes, and to improve the bonding power of the asphalt and the abrasion resistance of asphaltic compositions formed of asphalt and mineral aggregates, for example, sand and rock.

This invention is a result of extensive and continuing research into the chemical constitution of asphalts and into the chemistry of the weathering process of asphaltic pavements and other asphaltic compositions.

This application is a continuation-in-part of application 254,399, filed January 28, 1963, now abandoned and of application Serial No. 45,023, filed July 25, 1960, now abandoned, which in turn is a continuation in part of application 497,397, filed March 28, 1955, now abandoned.

Asphalts are generally understood to comprise non-distillable and high-boiling residues of petroleum fractions, consisting of asphaltenes, that is, components which are insoluble in n-pentane and of maltenes, i.e., fractions soluble in n-pentane.

Asphalts also include natural asphalts found as such, as deposits in the earth or produced from petroleum crude oils by distillation, or from cracked petroleum fractions. Asphalts are also produced by blending such residues with liquid petroleum oil fractions and also by blending such petroleum oil fractions with residues precipitated from the above asphalts by solvents, such as liquid propane.

Asphalts come in various grades, classified according to their penetration values, as is well known in the asphalt art. Paving grade asphalts are understood to include those asphalts usually produced by reduction of petroleum fractions, by steam distillation or vacuum distillation, or blending oils with natural, precipitated or reduced asphalts from petroleum oils, which have a penetration value of 32 or more, for example 200–300 (5", 100 gms.) [Test T49-49, American Association of State Highway Officials].

Other grades include roofing asphalts and other well recognized grades of asphalts derived from petroleum or from similar natural deposits.

The pentane soluble components, i.e., maltenes, have been identified and named as follows: The nitrogen bases, symbolized by the letter N; the Group I unsaturates, called first acidaffins, identified by the symbol A<sub>1</sub>; the Group II unsaturates, also known as second acidaffins, identified by the symbol A<sub>2</sub>; and the saturated fraction, also known as the paraffins fraction, identified by the letter P. The asphaltenes are identified by the letter A.

The method of analysis by which each one of these groups may be determined is described in "Compounding Rubber with Petroleum Products," by Rostler and Sternberg, published in Industrial and Engineering Chemistry, vol. 41, at pages 598–608, of March, 1949. The method has been further described in "Composition and Changes in Composition of Highway Asphalts, 85–100 Penetration Grade," published in proceedings of Association of Asphalt Paving Technologists, vol. 31, January 1962, at pages 72–79. This method of analysis and the terminology have been adopted in governmental specifications of high boiling oils, as recorded in the report of the work done in the Government laboratories in the Univer-

2

sity of Akron, Ohio, in the article entitled, "Oil Types in the Program for Oil Extended Rubbers," by Taft, et al., Industrial and Engineering Chemistry, 1955, vol. 47, pages 1077–1090. The method has further been adopted as an A.S.T.M. Procedure under the designation D-2006-62T.

The discussion of the method is also described in the article entitled, "Influence of Chemical Composition of Asphalts on Performance and Particularly Durability," by Rostler and White, in the American Society for Testing Materials' Special Publication No. 277, at pages 64–88.

This method identifies the components of asphalts and petroleum fractions having an initial boiling point not lower than 160° C., at 10 mm. Hg absolute pressure, previously described: asphaltenes, nitrogen bases, first acidaffins, second acidaffins and paraffins.

Throughout this application, wherever the terms "asphaltenes," "nitrogen bases," "first and second acidaffins," 20 also identified as "Group I or Group II unsaturates," and "paraffins" are used, it will be understood that they refer to the fractions as determined by the above analytical procedure.

In application Serial No. 497,397, I grouped the nitrogen bases and the Group I and Group II unsaturates in the term "resinous components" of the asphalt.

Application Serial No. 497,397 reports the discovery that the weathering produces an increase in the asphaltenes content, and that the total percentage of the resinous components decreases. The change appears explainable by the fact that the Group I unsaturates and nitrogen bases change into asphaltenes with a reduction in the bonding power of the asphalt. The result of weathering is to cause an unbalance as between the saturated fractions, on the one hand, and the resinous components, on the other hand. The application also describes the discovery that weathered asphalts may be rejuvenated by establishing the proper balance between the resinous components and the paraffins in the rejuvenated asphalt.

40 The process of the above application rejuvenated the weathered asphalt by reestablishing the balance of components, as it existed in the original asphalt before weathering. This is accomplished by adding fractions of maltenes which modify the composition of the weathered asphalt by the addition of sufficient resinous material to raise the content of the resinous component of the weathered asphalt so that the balance of components found in the original asphalt may be re-established. The maltenes added contain the resinous components, that is, the 45 nitrogen bases, and first and second acidaffins, in amounts of at least 50% by weight of the maltenes. The added maltenes may also contain saturated components, i.e., the paraffins.

The maltenes are preferably added to the weathered asphalt in emulsion form. The amount of maltenes added to the weathered asphalt is sufficient to materially improve the properties of the asphalt which, by weathering, has had its usefulness markedly reduced, as evidenced by the low penetration value and brittleness of the weathered 50 asphalt. The maltenes added to the weathered asphaltic pavement may be in amounts to bring the asphalt content of the pavement up to 1.3 to 1.4 times the amount specified for that pavement, for example, about 4% to 8% by weight of the asphaltic aggregate composition constituting 55 the pavement.

The aforesaid application is herewith incorporated by this reference.

Subsequent to the filing of the above application, my continued research into the subject developed further discoveries, including the effect of the composition on the durability of asphalts, as indicated by the abrasion resistance, using test procedures adopted by the Materials and

Research Department of the California Division of Highways, as described by F. N. Hveem in the Proceedings of the Association of Asphalt Paving Technologists, Technical Section, December 1, 1943, vol. 15, page 111, et seq.; and by John B. Skog, A.S.T.M. Special Technical Publication 212, page 1, et seq. The test consists of mixing two parts of asphalt with 100 parts of Ottawa sand at various temperatures and determining the abrasion loss by impinging a stream of steel shot against a compacted specimen. Additional samples are made in the same manner and exposed in a weathering machine to infrared heat for various times, and weathered samples withdrawn at various intervals and likewise tested. The parameter reported is grams loss per 1,000 gram shot. This test is herein referred to as the "Shot Abrasion Test."

Experience with this test has shown that the higher the abrasion loss by this test, after weathering, the inferior is the life expectancy of the road produced from these asphalts. (See the Skog article, page 8.) It is thus a measure of the durability of the asphalt, i.e., its resistance to loss of bonding properties and other characteristics which are useful in pavements.

Discoveries made in connection with this continued research are disclosed in my application, Serial No. 45,023. Data are reported as a result of this continued investigation by the applicant upon 200 to 300 penetration grade asphalt produced from California crude oils derived from the Los Angeles basin, Valley and Santa Maria fields in California. Thirteen such asphalts are reported in the aforesaid application. Additional data are reported for asphalts produced from California crude oils and from blends produced from Gilsonite and various oil fractions. The asphalt blends had penetration values in the range of 200-300, and the Gilsonite asphalts had penetrations ranging from 85 to 257.

These asphalts were subjected to the above tests, and the data showed that the abrasion resistance measured by the Shot Abrasion Test increases with an increase in the paraffins content (P) of the asphalt in a regular manner. The results of these experiments showed that, in order to obtain an asphalt of penetration from about 30 to about 300, having a loss of under 3 grams in the above Shot Abrasion Test after 500 hours' weathering, the percent paraffins in the asphalt should be above about 15%, and up to about 50%; and the higher the percentage in this range, the more abrasion resistant the asphalt.

The effects of weathering have been shown in application Serial No. 45,023 to result from an unbalance in the asphaltenes and saturated fractions on the one hand, and the unsaturated and nitrogen bases components on the other. The effect of unbalance is the lesser, the greater the percentage of saturated fractions in the asphalt originally employed.

The application Serial No. 45,023 taught that asphalts may be rejuvenated by adding the paraffins fractions to obtain the required balance to produce an asphalt of desirable properties. The percent of resinous fractions has, however, to be high enough to prevent syneresis. It is to be observed that maltenes employed may also contain the unsaturated fractions and may also contain nitrogen bases.

With some weathered asphalts, which are relatively uncommon, which are unusually high in peptizing fractions, to wit, the nitrogen bases and other resinous fractions, to wit: first and second acidaffins, the maltenes may be substantially all paraffins, i.e., higher than 85% and even 100%. In the cases which are normally encountered, I found that a weathered asphalt which has deteriorated may be suitable for the purpose of the structure in which it is used, if the weathered asphalt is plasticized by adding thereto the selected fractions of maltenes, containing a suitable concentration of the components in which the asphalt is deficient. Such fractions may be produced from petroleum oils by removing asphaltenes and wax of the oil, if the oil is a waxy oil, to produce fractions

containing about 20% to 85% saturated components, the remainder being reactive components, to wit: nitrogen bases and first and second acidaffins.

The application, Serial No. 45,023, further discloses data which show that the durability of rejuvenated asphalt is the greater the greater the percent paraffins (P), and that by increasing the paraffins content of the original asphalt employed in the road construction, the durability, as measured by the Shot Abrasion Test, at various stages of weathering was above that of the original asphalt, the abrasion loss being markedly reduced.

The results of the discoveries as reported in application Serial No. 45,023, therefore, showed that the addition of maltenes containing sufficient paraffins fractions (P), in amount sufficient to raise the paraffins content of a weathered asphalt, could produce an asphalt of bonding power and durability even better than that of the unweathered, original asphalt.

As disclosed in the said application, Serial No. 45,023, the fractions of maltenes are used in emulsion form, preferably as a cationic emulsion, and preferably also as a balanced emulsion containing both cationic and nonionic emulsifiers.

The aforesaid application, Serial No. 45,023, is hereinafter incorporated by this reference.

Continued research and investigation in this field resulted from the opportunity afforded applicant to investigate 119 asphalts obtained from crude oils produced in various states of the United States and in Venezuela, in Canada and in Mexico, and produced by various methods, including steam distillation, air blowing, blending, propane fractionation, and fluxing with heavy oils. The details of the test data upon these various asphalts and their origins are given in "Public Roads" of August 1959, vol. 30, No. 9, issued by the Department of Commerce, United States Government, pages 197-207, and also in the "Proceedings of the Association of Asphalt Paving Technologists," vol. 28, January 1959, pp. 242-279.

Samples of these asphalts were secured, and the samples were analyzed according to the analytical procedures given in the above method by Rostler and Sternberg and by a weathering and abrasion test method reported in the article entitled "Influence of Chemical Composition of Asphalts on Performance, Particularly Durability," by Rostler and White, published in American Society for Testing Materials, Special Technical Publication No. 277, pages 64-88, 1959. This abrasion test method, which, as shown in the article (see infra) "Composition and Changes in Composition of Highway Asphalts, 85-100 Penetration Grade," correlates with the Shot Test, will herein be referred to as the Pellet Test.

This investigation confirmed the results reported in application Serial No. 45,023, and showed that, as a general rule, the asphalts show greater abrasion resistance and durability to weathering, the higher the paraffins content, provided the paraffins content is not so high as to destroy the suitability of the asphalt as a bonding agent. It also explains and reconciles the results of the two previous applications, and shows that while in each case an improvement in the asphalt is obtained by following the procedures of the aforesaid applications, they are each a special case of a more general principle which makes it possible to improve the durability of asphalts, both weathered and unweathered.

The reason that this is so, as now appears from my further investigation, is that, as the paraffins content (P) of the asphalt increases, so is there an increase in the sum of the paraffins and second acidaffins ( $A_2$ ), and that the controlling factor is the ratio of the sum of the nitrogen bases and the first acidaffins ( $N+A_1$ ) to the sum of the paraffins and the second acidaffins ( $P+A_2$ ), expressed as the ratio of the percentages present in the asphalt. It thus appears that the reason that the asphalts of higher paraffinic content show a greater abrasion resistance and increased durability is that this ratio decreases as the

concentration of paraffins increases. However, the paraffins content is not as sensitive an indicator for durability of many asphalts with paraffins contents in excess of about 10% to 15%. The above maltenes composition ratio  $N+A_1/P+A_2$ , is thus a better and more sensitive index of the durability of the asphalt than the content of the component P.

Asphalts investigated by means of the Pellet Test, including the 119 asphalts and two other asphalts of 85 to 100 penetration grade (Samples No. 19 and 20 of Table III) which were blended to have an excessively low ratio, showed that the asphalts vary in their maltenes composition ratio from about .3 to above 2, and have abrasion losses by the above Pellet Tests ranging from no loss, or zero loss, to about 100%. These asphalts may be classified into various groups, according to their loss on abrasion by the above Pellet Tests, taken as the average of the abrasion loss before and after aging, as shown in Table I.

characteristics. On top of FIGURE 1 is indicated the boundaries of the groups corresponding to values of the ratio for each group, plotted as abscissa.

Line D on FIGURE 4 and the same data plotted as a curve on FIGURE 2 plot the paraffins content of the groups of Table I against the same average abrasion loss.

The above tests show that, for the 85-100 penetration asphalts produced by various procedures from petroleum crude oils of various types and diverse geographic origins, the following conclusions may be drawn:

For asphalts with paraffins content ranging from about 7% to about 40%, and asphaltenes content ranging from about 11% to 36%, the abrasion loss is a function of the ratio of  $N+A_1/P+A_2$  as well as of the paraffins content. It also appears that, for abrasion loss in excess of about 20%, the above ratio is a much more sensitive index of the durability of the asphalt than is the percent paraffins.

TABLE I

| Durability Group | $\frac{N+A_1}{P+A_2}$ |         | Average*<br>Percent<br>Paraffins | Average**<br>Abrasion | Durability Rating                                      |
|------------------|-----------------------|---------|----------------------------------|-----------------------|--------------------------------------------------------|
|                  | Range                 | Average |                                  |                       |                                                        |
| 0-----           | <0.4                  | 0.28    | 39.8                             | 50                    | Decreasing durability with decreasing parameter value. |
| I-----           | 0.4 to 1.0            | 0.82    | 13.8                             | 5.7                   | Superior.                                              |
| II-----          | 1 to 1.2              | 1.09    | 11.5                             | 8.9                   | Good.                                                  |
| III-----         | 1.2 to 1.5            | 1.34    | 9.9                              | 29.6                  | Satisfactory.                                          |
| IV-----          | 1.5 to 1.7            | 1.58    | 8.9                              | 45.4                  | Fair.                                                  |
| V-----           | >1.7                  | 1.84    | 9.0                              | 52.7                  | Inferior.                                              |

\* Composition of original (nonaged) asphalt.

\*\* Average of percent abrasion (Pellet Method) before and after 7 days aging.

FIGURES 1-5 are plots of data given in this specification.

FIGURE 1 shows the average abrasion loss by the Pellet Test plotted against the composition ratio  $N+A_1/P+A_2$  of the original unaged asphalt. The average abrasion loss is calculated as the average of the abrasion loss of the unaged mixture of Ottawa sand and asphalt, and the same mix, after aging seven days as described in the above article by Rostler and White in the article in vol. 31 of the Proceedings of the Association of Asphalt Technologists, supra and A.S.T.M. Special Technical Publication No. 277.

The solid curve is drawn as a best fit to the data obtained from the above 85-100 penetration grade asphalts, and the dotted line gives the trend line for asphalts of composition ratios in the various groups.

The marked points where the ratio is .4 and less are for asphalts sample Nos. 10 and 20, ab above. All other points are averages as given in Table I. The asphalts fall into six groups. Group 0, with composition ratios less than 0.4, represents compositions which are of consistency of a chessy and putty-like character rather than asphalts. At about 0.4 the compositions attain the desirable characteristic of paving grade asphalts.

The asphalts of Groups I to V may be rated as stated in the table, based on their durability. The lower the abrasion loss initially, and also the less abrasion loss after aging, the better is the asphalt, i.e., the lower the above average, the better the asphalt in its weathering

The following asphalts had the values expressive of composition given in the following Table II:

TABLE II

| Sample No. | Initial Composition |                         | $\frac{N+A_1}{P+A_2}$ | Abrasion Loss* |
|------------|---------------------|-------------------------|-----------------------|----------------|
|            | Percent Par. (P)    | Percent Asphaltenes (A) |                       |                |
| 55         |                     |                         |                       |                |
| 1-----     | 16.6                | 8.8                     | 1.16                  | 8              |
| 2-----     | 16.2                | 9.2                     | 1.22                  | 6              |
| 3-----     | 16.2                | 26.6                    | 1.36                  | 9              |
| 4-----     | 15.5                | 10.5                    | 1.23                  | 9              |
| 5-----     | 15.1                | 11.6                    | 1.47                  | 12             |
| 6-----     | 15                  | 12.4                    | 1.58                  | 16             |
| 7-----     | 14.7                | 9.5                     | 1.33                  | 9              |
| 8-----     | 14.3                | 21.7                    | 1.41                  | 10             |
| 9-----     | 13.4                | 17                      | 1.61                  | 20             |
| 10-----    | 12.5                | 25.7                    | 1.41                  | 15             |
| 11-----    | 12.4                | 14.9                    | 1.89                  | 12             |
| 12-----    | 12.2                | 24.6                    | 1.48                  | 15             |
| 13-----    | 11.6                | 25.6                    | 1.77                  | 20             |
| 14-----    | 21.3                | 9.2                     | 1.14                  | 4              |
| 15-----    | 19.1                | 7.2                     | 1.24                  | 5              |
| 16-----    | 11.9                | 8.4                     | 1.48                  | 8              |
| 17-----    | 10.4                | 4.0                     | 1.35                  | 8              |
| 18-----    | 4.6                 | 1.5                     | 6.2                   | 30             |

\* Determined by the Shot Abrasion Test on Samples after weathering for 500 hours in the weathering machine.

The asphalts of Samples 1-13 were all 200-300 penetration grade asphalt. The table gives the percent paraffins (P), and the percent asphaltenes (A), and the ratio  $N+A_1/P+A_2$ .

Samples 14-18 were all made by blending 32 penetration asphalt with various oil fractions to give a 200-300 penetration asphalt as follows:

Sample:

|    |                        |    |
|----|------------------------|----|
| 14 | 83%, asphalt, 17% oil. | 5  |
| 15 | 73% asphalt, 27% oil.  |    |
| 16 | 73% asphalt, 27% oil.  | 15 |
| 17 | 45% asphalt, 55% oil.  |    |
| 18 | 20% asphalt, 80% oil.  | 10 |

The 32 penetration asphalt had the following composition:

|                   |         |      |
|-------------------|---------|------|
| Asphaltenes       | percent | 1.34 |
| Nitrogen bases    | do      | 41.7 |
| First acidaffins  | do      | 13.9 |
| Second acidaffins | do      | 19.3 |
| Paraffins         | do      | 11.7 |
| $N+A_1/P+A_2$     |         | 1.82 |

The oil employed in Sample 14 was 50SAE heavy raffinate which had the following composition:

|                   |         |      |
|-------------------|---------|------|
| Nitrogen bases    | percent | 3.4  |
| First acidaffins  | do      | 6.5  |
| Second acidaffins | do      | 28.0 |
| Paraffins         | do      | 62.1 |
| $N+A_1/P+A_2$     |         | 1.11 |

It had the following distillation range at 10 mm. Hg pressure:

|                       |    |     |    |
|-----------------------|----|-----|----|
| Initial boiling point | °C | 244 | 30 |
| 50% point             | °C | 322 |    |
| End point             | °C | 385 |    |

The blended asphalt had the following composition:

|                   |         |      |    |
|-------------------|---------|------|----|
| Asphaltenes       | percent | 9.2  | 35 |
| Nitrogen bases    | do      | 36.7 |    |
| First acidaffins  | do      | 11.7 |    |
| Second acidaffins | do      | 21.1 |    |
| Paraffins         | do      | 21.3 |    |
| $N+A_1/P+A_2$     |         | 1.14 | 40 |

Sample 15 was formed using S.R. stock, 154 Universal Saybolt Seconds at 210° F.

The S.R. stock had the following composition:

|                   |         |      |
|-------------------|---------|------|
| Nitrogen bases    | percent | 14.6 |
| First acidaffins  | do      | 14.3 |
| Second acidaffins | do      | 35.4 |
| Paraffins         | do      | 35.7 |
| $N+A_1/P+A_2$     |         | 0.41 |

It had substantially the same distillation range as the S.A.E. 50 used in Sample 14.

The asphalt composition of the asphalt in Sample 15 was:

|                   |         |      |
|-------------------|---------|------|
| Asphaltenes       | percent | 7.2  |
| Nitrogen bases    | do      | 37.4 |
| First acidaffins  | do      | 14.0 |
| Second acidaffins | do      | 22.3 |
| Paraffins         | do      | 19.1 |
| $N+A_1/P+A_2$     |         | 1.24 |

Sample 16 was made using 27% Medium Lubricating Extract having the following composition:

|                   |         |      |
|-------------------|---------|------|
| Nitrogen bases    | percent | 17.3 |
| First acidaffins  | do      | 17.3 |
| Second acidaffins | do      | 53.0 |
| Paraffins         | do      | 12.4 |
| $N+A_1/P+A_2$     |         | .53  |

It had the following distillation range at 10 mm. Hg pressure:

|                       |    |     |
|-----------------------|----|-----|
| Initial boiling point | °C | 205 |
| 50% point             | °C | 263 |
| End point             | °C | 295 |

The blended asphalt in Sample 16 had the following composition:

|                   |         |      |
|-------------------|---------|------|
| Asphaltenes       | percent | 8.4  |
| Nitrogen bases    | do      | 35.2 |
| First acidaffins  | do      | 19.5 |
| Second acidaffins | do      | 25.0 |
| $N+A_1/P+A_2$     |         | 1.48 |
| Paraffins         | percent | 11.9 |

Sample 17 was made using 55% Heavy Lubricating Oil Extract having the following composition:

|                   |         |      |
|-------------------|---------|------|
| Nitrogen bases    | percent | 28.7 |
| First acidaffins  | do      | 21.2 |
| Second acidaffins | do      | 41.3 |
| Paraffins         | do      | 8.8  |
| $N+A_1/P+A_2$     |         | 0.99 |

It had substantially the same distillation range as the S.A.E. 50 used in Sample 14.

The blended asphalt in Sample 17 had the following composition:

|                   |         |      |
|-------------------|---------|------|
| Asphaltenes       | percent | 4.0  |
| Nitrogen bases    | do      | 36.4 |
| First acidaffins  | do      | 18.7 |
| Second acidaffins | do      | 30.5 |
| Paraffins         | do      | 10.4 |
| $N+A_1/P+A_2$     |         | 1.35 |

Sample 18 was made by blending with a concentrate of nitrogen bases having the following composition:

|                   |         |      |
|-------------------|---------|------|
| Nitrogen bases    | percent | 84.6 |
| First acidaffins  | do      | 7.3  |
| Second acidaffins | do      | 6.7  |
| Paraffins         | do      | 1.4  |
| $N+A_1/P+A_2$     |         | 11   |

The blended asphalt had the following composition:

|                   |         |      |
|-------------------|---------|------|
| Asphaltenes       | percent | 1.5  |
| Nitrogen bases    | do      | 77   |
| First acidaffins  | do      | 7.8  |
| Second acidaffins | do      | 9.1  |
| Paraffins         | do      | 4.6  |
| $N+A_1/P+A_2$     |         | 6.12 |

The above distillation range and boiling points are determined by A.S.T.M. Test D-1160.

FIGURE 4 shows, in addition to line D discussed above, the relation of percent paraffins to abrasion loss given in Table II for the asphalt Samples 1 to 13 and also for Samples 14 to 18. The lines are given only to indicate the trend of the dependence of abrasion resistance on percent paraffins and are not intended to imply a mathematical law.

FIGURE 3 shows the relation of the composition ratios of the asphalts of Table II to the abrasion loss by the Shot Abrasion Test after weathering for 500 hours.

As in the case of 85-100 penetration grade asphalts, whose averages are plotted on FIGURE 1, the asphalts of 200-300 penetration grade also show the dependence of abrasion loss on the composition ratio. Notwithstanding the differences in the methods of testing the abrasion loss and resistance to weathering, both tests show that an increase in the ratio  $N+A_1/P+A_2$  results in a decrease in the durability of the asphalt as measured by either test.

Asphalts produced by blending Gilsonite with an oil also show a reduction in abrasion loss with increasing paraffins content and decreasing  $N+A_1/P+A_2$  composition ratio. They illustrate, however, the additional fact that an excessively low ratio, substantially below a ratio

of about 0.4, indicating an excessively high concentration of paraffins and second acidaffins, reduces the bonding power and results in a relatively high abrasion loss.

The following table illustrates this phenomenon:

300 penetration grade also gave abrasion loss of under 50 grams.

Thus, asphalts of superior abrasion resistance are those whose composition ratios are more than about 0.4, and

TABLE III

| Sample | Composition, percent by Wt. |      |      |      |                    |          | Abrasion Loss              |                     |
|--------|-----------------------------|------|------|------|--------------------|----------|----------------------------|---------------------|
|        | Gilsonite                   | Oil  | P-   | A    | $N+A_1$<br>$P+A_2$ | Penetra- | Shot<br>Abrasion<br>Test 1 | Pellet<br>Average 2 |
| 19     | 38.5                        | 61.5 | 39.8 | 26.1 | 0.29               | 85       | 1                          | 50                  |
| 20     | 41                          | 59   | 7.1  | 29.9 | 0.4                | 85       | 27                         | 11                  |
| 21     | 16.5                        | 83.5 | 1.9  | 9.9  | 10                 | 87       | 86                         | 100                 |
| 22     | 35                          | 65   | 43.4 | 24.3 | .24                | 134      | 0                          | 50                  |
| 23     | 37                          | 63   | 7.9  | 25.7 | .37                | 132      | 10                         | 1                   |
| 24     | 11                          | 89   | 1.5  | 6.7  | 11.8               | 149      | 57                         | 100                 |
| 25     | 31.5                        | 68.5 | 44.5 | 20.1 | .22                | 229      | 0                          | 0                   |
| 26     | 84                          | 66   | 8.7  | 21.8 | .32                | 249      | 4                          | 1                   |
| 27     | 3                           | 97   | 1.5  | 1.6  | 11                 | 257      | 37                         | 40                  |

<sup>1</sup> Specimen aged in weathering machine before test.

<sup>2</sup> Average of percent abrasion before and after 7 days' aging.

The data confirm the observations discussed above that for unweathered asphalts (asphalts containing 40% or less of paraffins and having ratios of 0.4 or higher), the durability, as measured by either the Shot Abrasion Test or the Pellet Test, as abrasion loss, increases with increase in the percent paraffins, and that asphalts with ratios of from 0.4 to 1.15 have abrasion losses by the Pellet Test of under 10%, and the abrasion loss increases rapidly with increase of ratio beyond 1.15.

The data show that, as a conservative measure, until further research fixes the effect of paraffins content in excess of 40% and ratios  $N+A_1/P+A_2$  of less than 0.4, the desirable composition of unweathered asphalts to give superior durability, I conclude, are those having paraffins content of less than about 40% and ratios  $N+A_1/P+A_2$  of more than about 0.4, and the asphalts of ratios from about 0.4 to about 1.5 will all have satisfactory durability. Asphalts of the 85-100 penetration grade with ratios above about 1.5 rapidly lose in abrasion resistance as the ratio increases.

It is, therefore, one object of my invention to improve asphalts, which are produced from a petroleum crude or a fraction thereof by distillation or blending an asphalt of relatively low penetration with maltenes, and which asphalts show a high abrasion loss and low durability, by adding to the asphalt a petroleum fraction which will adjust its ratio of  $N+A_1/P+A_2$  to be within the desirable range. For asphalts of lower than about 100 penetration, the said desirable range is above 0.4 and less than its original ratio, if above about 1.5.

Experience has shown that, for 85-100 penetration paving grade asphalt, it is desirable for superior performance in the field that the abrasion loss by the Shot Abrasion Test be not over 50 grams/1,000 grams of shot after weathering for 500 hours, and preferably should be much lower; and that the lower the abrasion loss by this test, the more durable is the asphalt. Pavements made of asphalt of 20 grams loss or less will last longer than those which show 30 grams loss or higher, since the bonding power of the asphalts of 30 grams loss appear impaired as compared with the asphalt of 20 grams loss.

As will appear from FIG. 3, for 200-300 penetration grade asphalts, asphalts of ratio less than 1.35 will have an abrasion loss of less than 10 grams for the Shot Abrasion Test after aging for 500 hours, and asphalts of ratio less than 1.7 will have an abrasion loss of less than 20 grams by the Shot Abrasion Test after aging for 500 hours. From Table II (see Sample 18) the ratio may be substantially higher and give abrasion losses under 50 grams, and, as will be seen in the case of the Gilsonite blends of Table III, ratios of as high as 11 for the 200-

25 the upper limit of ratio for asphalts with good abrasion resistance depends on the penetration grade of the asphalt. For asphalts of 100 or less penetration, the upper limit is suitably about 1.5, and for softer asphalts the ratio may be higher. Thus, in the penetration grade 200-300, the ratio is suitably less than 10. Also, the paraffins content is preferably below about 40% of the asphalt.

30 The abrasion loss of asphalts may be improved by incorporating, into the asphalt of relatively high ratio and relatively high abrasion loss, fractions in quantity and amount to adjust the ratio to the desired value. Since 35 this will cause some increase in the penetration value of the asphalt, it may be necessary, if the attained penetration is undesirable, to either start with a low penetration asphalt, or employ as the blending oil an oil which has a high value of its  $P+A_2$  fraction, minimizing the total amount of maltenes which is introduced.

30 The following illustrates the effect of the concentration of the above fractions in the asphalt to be improved and of the oil used for the improvement.

40 If  $N+A_1$  and  $P+A_2$  are the concentrations of these fractions in the asphalt to be improved, and  $R_a$  is their ratio  $N+A_1/P+A_2$ ;

45 And  $N'+A'_1$  and  $P'+A'_2$  are the concentrations of these fractions in the oil to be added, and  $R_o$  is their ratio  $N'+A'_1/P'+A'_2$  in the oil employed;

50  $R$  is the desired ratio which is to be attained for the asphalt to be improved.

55  $Z$  is the ratio of the weight of the oil to be employed to the weight of asphalt to be treated.

Let

55  $x$  = weight of the asphalt;  
 $y$  = weight of the oil;

$$y/x = Z$$

$$\frac{(N+A_1)x+(N'+A'_1)y}{(P+A_2)x+(P'+A'_2)y} = R$$

60 Dividing by  $x$ :

$$R = \frac{(N+A_1)+(N'+A'_1)Z}{(P+A_2)+(P'+A'_2)Z}$$

$$Z = \frac{(N+A_1)-R(P+A_2)}{R(P'+A'_2)-(N'+A'_1)}$$

$$Z = \frac{(P+A_2)(R_a-R)}{(P'+A'_2)(R-R_o)}$$

70 The composition of the oil to be added will depend on the amounts of maltenes which may be added to obtain the desired penetration grade. This depends on the penetration value of the asphalt which it is desired to improve and the penetration value which is desired in the improved asphalt. It appears from the foregoing that the

higher the concentration of the fractions  $P+A_2$  the less of the oil is necessary to obtain the reduction of the ratio R to a target value. The composition and the amount employed are regulated so as to produce an improved asphalt of desired penetration value, with a paraffins content less than about 40% and a ratio R of more than about 0.4.

The previous examples illustrate the nature and amount of the maltenes which may be employed for the 85-100 penetration grade asphalt.

Using the above equations, the amount of maltenes to be added may be calculated, if the composition of the asphalt to be improved and the composition of the maltenes to be added are known, and the desired value of R is specified.

It is an object of my invention to shift the composition ratio to a value closer to 0.4 than the value of the asphalt to be improved, which should be sufficiently reduced or raised in value to result in a substantial increase in the abrasion resistance.

Where the asphalt to be improved has a ratio substantially less than 0.4, I employ an oil having a ratio substantially higher than the ratio of the asphalt, preferably a ratio of 0.4 or higher. Where the asphalt to be improved has an excessively high ratio, I employ an oil having a substantially lower ratio.

By using maltenes of a ratio of about 0.4, I may improve asphalts of higher or lower ratio without first determining the ratio of the asphalt, since if the ratio of the asphalt is in excess of 0.4, the oil will reduce the ratio but not to or below 0.4. In treating asphalts of excessively low ratios, the 0.4 ratio maltenes will raise the ratio of the asphalt towards 0.4 and thus also improve the asphalt.

TABLE IV

| Sample | 32 Pen. Asphalt |                | Maltenes    |                | Improved Asphalt |      | Shot Abrasion Test, Loss After 500 hrs. |  |
|--------|-----------------|----------------|-------------|----------------|------------------|------|-----------------------------------------|--|
|        | Composition     |                | Composition |                | Composition      |      |                                         |  |
|        | P               | R <sub>a</sub> | P           | R <sub>a</sub> | P                | R    |                                         |  |
| 14     | 13.4            | 1.84           | 62.1        | 0.11           | 21.3             | 1.14 | 4                                       |  |
| 15     | 13.4            | 1.84           | 35.7        | 0.41           | 19.1             | 1.24 | 5                                       |  |
| 16     | 13.4            | 1.84           | 12.4        | 0.53           | 11.9             | 1.48 | 8                                       |  |
| 17     | 13.4            | 1.84           | 8.8         | 0.99           | 10.4             | 1.35 | 8                                       |  |
| 18     | 13.4            | 1.84           | 1.4         | 11             | 4.6              | 6.2  | 30                                      |  |

The above Table IV illustrates the effect of the R<sub>a</sub> value of the oil. It is apparent that the oil should have an R<sub>a</sub> value less than that of the asphalt to be improved, and preferably the lower this value the better; but the amount employed, and the paraffinic content, and the R<sub>a</sub> value of the oil should not raise the paraffinic content and lower the R value to undesirable limits, as stated above.

The oils should also be relatively high boiling petroleum fractions and substantially free of fractions boiling below about 160° C. at 10 mm. Hg absolute pressure, and preferably should have a distillation range whose initial value is about 200° C. at 10 mm. Hg absolute pressure (A.S.T.M. Test D-1160). It has been found that employing the lower boiling oils (notwithstanding they be of composition and be used in amounts to produce the desirable paraffins content, R ratio and penetration) produces asphalts of inferior durability according to the above tests. This is illustrated by the following data.

Sample 28 was made by blending the 32 penetration asphalt used in producing Samples 14-18. It was blended with a light spray oil extract in the following ratios by weight: 87.5% of the asphalt and 12.5% of the light spray oil extract. The spray oil extract had the following composition:

Nitrogen bases percent 5.9  
First acidaffins do 14.6  
Second acidaffins do 58.8

Paraffins do 20.7  
N+A<sub>1</sub>/P+A<sub>2</sub> do 0.258

The oil had the following distillation range:

Initial ° C. 170  
50% ° C. 229  
End point ° C. 253

The blended asphalt had the following composition and properties:

Asphaltenes percent 11  
Nitrogen bases do 38.7  
First acidaffins do 15.6  
Second acidaffins do 21.5  
Paraffins do 13.2  
N+A<sub>1</sub>/P+A<sub>2</sub> 1.56  
Abrasion loss, Shot Abrasion Test 41.8

This may be compared with Sample 16 above, in which a medium lubricating oil extract was employed to give an asphalt of similar composition, both as to paraffins content as well as R value, and both having a ratio of about 1.5.

A similar result is obtained by employing a technical white oil (98% unsulfonated residue) of 100 Saybolt Seconds at 100° F.

Sample 29 was produced by blending 89% by weight of the above 32 penetration asphalt with 11% by weight of the above technical white oil.

The white oil had the following composition:

Nitrogen bases percent 0  
First acidaffins do 0.1  
Second acidaffins do 5.3  
Paraffins do 94.6  
N+A<sub>1</sub>/P+A<sub>2</sub> 0.01

The distillation range was the same as for the spray oil extract of Sample 28.

The resultant asphalt had the following composition and abrasion loss by the Shot Abrasion Test:

Asphaltenes percent 10.4  
Nitrogen bases do 38.4  
First acidaffins do 12.7  
Second acidaffins do 18.2  
Paraffins do 20.3  
N+A<sub>1</sub>/P+A<sub>2</sub> 1.33  
Abrasion loss 23.5

This may be compared with Sample 15, which resulted in an asphalt of similar composition, both in paraffins content and ratio. These results are tabulated below.

TABLE V

| Sample | Maltenes    |                                 |   |               | Asphalt     |            | Shot Abrasion Test Loss |  |
|--------|-------------|---------------------------------|---|---------------|-------------|------------|-------------------------|--|
|        | Composition | Distillation Range <sup>1</sup> |   |               | Composition |            |                         |  |
|        |             | P                               | R | Initial, ° C. | 50%, ° C.   | E.P., ° C. |                         |  |
| 28     | 20.7        | 0.26                            |   | 170           | 229         | 253        | 13.2 1.56 42            |  |
| 16     | 12.4        | 0.53                            |   | 205           | 263         | 295        | 11.9 1.48 8             |  |
| 29     | 94.6        | 0.01                            |   | 170           | 229         | 253        | 20.3 1.33 24            |  |
| 15     | 35.7        | 0.41                            |   | 244           | 322         | 385        | 19.1 1.24 5             |  |

<sup>1</sup> At 10 mm. (Hg) absolute pressure.

It thus appears that, even though the oil to be employed has sufficient concentrations of paraffins and also second acidaffins to have the desirable R ratio so that one may obtain the desired R ratio in the blended asphalt and give the desired penetration, it will not achieve the same low value of the abrasion loss if it contains volatile components so that its initial boiling point in the above tests is substantially below 160° C. at 10 mm. Hg pressure absolute. It should be preferably substantially free of fractions boiling below about 200° C. at such pressure. By "substantially

free," as used in this connection in the specification and claims, I means that the oil should not contain fractions boiling below about 200°, in amounts sufficient to result in an undesirable increase in abrasion loss.

The above observations were all related to the effect of the chemical composition of unweathered asphalts on the properties of the asphalt, particularly their durability when exposed to weathering as measured by the test procedures described above.

Studies in the behavior of asphalts during weathering and the changes which occur in chemical composition, and the beneficial effects of blending weathered asphalts with maltenes, have produced the following surprising results.

Two asphalts, identified as Asphalt A (same as Sample 18) and Asphalt B (same as Sample 16) were weathered, and the weathered asphalt was blended each with two different maltenes having different compositions.

The asphalt, after being subjected to weathering for 650 hours in the weathering machine, was tested for abrasion loss by the Shot Abrasion Test and analyzed. The weathered asphalt from A is given below as A', and the weathered asphalt from B is B'.

One portion was treated with an aqueous emulsion of maltenes containing 60% by weight of maltenes *a* (Method I), and another by a different maltenes *b* (Method II). This gave four asphalts. Asphalt A'*a* is the weathered A' asphalt treated with the maltenes *a* (Method I); A'*b* is the weathered A' asphalt treated with the maltenes *b* (Method II); B'*a* is the weathered B' asphalt treated with the maltenes *a* (Method I); B'*b* is the B' asphalt treated with the maltenes *b* (Method II). The asphalts so treated were again aged for 650 hours in the weathering machine and tested by the Shot Abrasion Test.

The composition of maltenes *a* employed in Method I and the maltenes *b* employed in Method II are given in the following table:

TABLE VI

|                                    | N,<br>percent | A <sub>1</sub> ,<br>percent | A <sub>2</sub> ,<br>percent | P,<br>percent | R    |
|------------------------------------|---------------|-----------------------------|-----------------------------|---------------|------|
| Maltenes <i>a</i> (Method I)-----  | 17            | 17                          | 54                          | 12            | 0.52 |
| Maltenes <i>b</i> (Method II)----- | 3.5           | 6.5                         | 28                          | 62            | 0.11 |

The emulsifier was a fatty quaternary ammonium salt 0.7% by weight (cationic emulsifier) and a non-ionic emulsifier (alkylphenylethylene oxide condensation product) 0.5% by weight of the emulsion.

The results are tabulated below.

TABLE VII

| Asphalt           | Asphalt Composition |     | Abrasion<br>loss |
|-------------------|---------------------|-----|------------------|
|                   | P                   | R   |                  |
| A-----            | 4.6                 | 6.1 | 1.37             |
| A' <i>a</i> ----- | 3.8                 | 4.7 | 2.53             |
| A' <i>b</i> ----- | 11.0                | 3.2 | 2.4              |
| B-----            | 11.9                | 1.5 | 1.8              |
| B' <i>a</i> ----- | 10.9                | 1.3 | 2.4              |
| B' <i>b</i> ----- | 15.5                | 1.2 | 2.1              |

<sup>1</sup> Weathered for 650 hours, Shot Abrasion Test.

<sup>2</sup> Aged an additional 650 hours after treatment.

Comparing Asphalt A, which on aging had an abrasion loss of 37 by the Shot method, with the Asphalt B, which showed 8, reveals the influence of the paraffins content and the R ratio, as previously explained.

This is also revealed by comparing the percent paraffins

and the R ratio of the asphalts A'*a*, A'*b*, B'*a* and B'*b* with their abrasion values. It also reveals that the asphalt with the higher R ratio and lower paraffins content shows the higher abrasion.

The low values of the abrasion losses for A'*b*, B'*a* and B'*b* are surprising. Thus, the improvement obtained employing maltenes *b* (Asphalt A'*b*) gave an asphalt with an abrasion value of 4. The increase in the durability of the asphalt reflects the increase in the paraffins content and reduction in the R ratio, although the increase in the durability is in excess of what would be expected for an unweathered asphalt. The same phenomenon appears with the B series. The reclaimed asphalts B'*a* and B'*b* both have relatively low values of R and show lower abrasion loss, the treated asphalt showing a better durability, i.e., lower abrasion loss, after treatment compared with the original asphalt.

I may rejuvenate weathered asphalts by incorporating into the asphalt petroleum fractions of such composition and amount as to reduce the R ratio of the asphalt, and can thus rejuvenate a weathered road and obtain a pavement having an even greater durability than when the road was freshly laid.

Field experience confirms this result. A road which had been weathered for two years was divided into three sections; one was as is, the second was treated with 0.11 gallon/square yard with the cationic maltenes emulsion described below, and the third was treated with 0.22 gallon/square yard of the same emulsion. The untreated section and the treated sections were cored to a  $\frac{3}{8}$ " depth, i.e., top or surface section; a second core was taken to a further depth of about 1", i.e., the middle section of the road. The cores were then extracted by the following procedure.

A sample of asphaltic paving material is first heated to a temperature of approximately 140° F. by any convenient means, as in an oven or over a steam plate. At this temperature most samples can be crumbled by hand. Extremely hard samples may require the use of pliers or a hammer. The sample should be reduced to about  $\frac{3}{4}$ " pieces or to the size of the largest pieces of aggregate, whichever is larger. Care should be taken not to break up the rocks and stones of the aggregate, so that the grading of the aggregate can be determined by sieve analysis on the sample after extraction.

The crumbled material is first weighed and then is placed into extraction thimbles of a Soxhlet extraction apparatus and covered with a loose plug of absorbent cotton to retain the aggregate. A thimble found suitable is a Whatman single thickness 43 x 123 mm. thimble. The asphalt is extracted in the Soxhlet apparatus with benzol until the benzol in the extraction chamber is colorless. The benzol extract is filtered as some of the finer aggregate passes through the single-thickness extraction thimbles. One may employ a 6-inch funnel using Whatman #1, 24 cm. filter paper or any other suitable filter. The benzol is distilled off from the extracted asphalt by heating the flask of the distilling apparatus in an electrically heated wax bath or oil bath at 150° C. Last traces of benzol are removed by carefully applying vacuum to the distilling apparatus while continuing to heat the flask in the wax bath at 150° C. The weight of the asphalt in the flask may be determined. This asphalt is herein referred to as extract asphalt.

The maltenes in the emulsion employed contained about 26% paraffins and had an  $R_0$  ratio of about .4. They were employed in a 2:1 ratio of concentrate to water. The emulsion concentrate contained 60% by weight maltenes and 0.9% of a cationic emulsifier (fatty amido-amino amine propionate, Promene 2115, Process Chemical Co.) and 0.9% of a nonionic emulsifier (dodecyl phenol polyethoxy ethanol, Pronon 280, Process Chemical Co.), and the balance water. This emulsion was employed in the tests hereinafter referred to, unless otherwise specified.

The results are tabulated in Table VIII.

TABLE VIII

| Core Identification                                              | Untreated |        | Treated (0.11 gsy) |        | Treated (0.22 gsy) |        |
|------------------------------------------------------------------|-----------|--------|--------------------|--------|--------------------|--------|
|                                                                  | Top       | Middle | Top                | Middle | Top                | Middle |
| Asphalt content, by Soxhlet Extraction, percent aggregate weight | 3.8       | 4.4    | 5.2                | 4.9    | 5.0                | 5.0    |
| Viscosity, megapoises                                            | 37.3      | 14.3   | 14.0               | 24.3   | 2.7                | 22.0   |
| Penetration Value, 0.1 mm.                                       | 17        | 26     | 26                 | 20     | 56                 | 22     |
| Chemical Composition (Rostler Method), Percent by Weight:        |           |        |                    |        |                    |        |
| Asphaltenes                                                      | 25.8      | 20.6   | 25.5               | 21.9   | 24.9               | 22.8   |
| Nitrogen Bases                                                   | 31.9      | 35.3   | 29.7               | 34.6   | 28.1               | 34.7   |
| First Acidaffins                                                 | 10.2      | 12.8   | 10.9               | 12.7   | 10.4               | 11.9   |
| Second Acidaffins                                                | 18.3      | 17.2   | 18.7               | 16.7   | 19.9               | 16.2   |
| Paraffins                                                        | 13.8      | 14.1   | 15.2               | 14.1   | 16.7               | 14.4   |
| Pellet Abrasion Test, Percent Loss in Weight:                    |           |        |                    |        |                    |        |
| As Recovered                                                     | 64        | 27     | 8                  | 42     | 1                  | 42     |
| Aged <sup>1</sup>                                                | 100       | 72     | 39                 | 88     | 4                  | 90     |
| Ratio (R): N+A <sub>1</sub> /P+A <sub>2</sub>                    | 1.31      | 1.34   | 1.20               | 1.54   | 1.05               | 1.52   |

<sup>1</sup> I.e., after weathering as reported in Rostler and White article.

The road surface after treatment was in excellent "live" condition.

The road test confirms the above results that a weathered asphalt may be improved and a weathered asphaltic structure may be reclaimed by adding petroleum fractions to increase the paraffins content, and particularly by adjusting the R ratio of the bonding asphalt.

It is thus an object of my invention to improve the weathering resistance of asphalts, whether originally weathered or unweathered, by treating the asphalt with a petroleum fraction to adjust the R ratio of the asphalt to reduce the R ratio if the R ratio is excessively high, for example, substantially above 1.5, or increase the R ratio if it is less than about 0.4, to a value in the range of about 0.4 to about 1.5.

The improvement attained in the road described above resulted from the reduction in R ratio by the treatment.

Where a weathered road contains weathered asphalt of excessively low R ratio, it may be reclaimed by treating the road by the application of a maltenes emulsion of a higher R ratio than that of the weathered asphalt. A road so treated was successfully reclaimed by this process, as illustrated by Example 6 given below.

As a rule, paraffins content is also increased by the treatment, but should not exceed about 40% of the asphalt.

I may employ any petroleum oil fraction, substantially free of asphaltenes, containing paraffins and containing members chosen from the group of the nitrogen bases, first acidaffins, and second acidaffins; that is, with or without the presence of one or more than one of the following: first acidaffins, second acidaffins or nitrogen bases. I may also employ oils containing second acidaffins with or without paraffins, first acidaffins or nitrogen bases. As a practical matter, petroleum oils will usually contain both paraffins and second acidaffins, and may also contain nitrogen bases and first acidaffins or one of the latter two members.

Such maltenes fractions may be produced from petroleum oils by removing the asphaltenes and wax of the oil (if the oil is a waxy oil) from the oil thereof to produce fractions which have about 5% to about 95% of paraffins components, with or without second acidaffins, the remainder being the more reactive components, to wit, the nitrogen bases and the first acidaffins, and having a R ratio of from less than 0.01 to about 19. Since the purpose of my invention is to add components chosen from the group of paraffins and second acidaffins and, if necessary, enough of the more reactive components, to wit, components chosen from the group of the nitrogen bases and first acidaffins, to peptize and dissolve the asphaltenes, I prefer to employ, as described above, a petroleum fraction which has the required concentrations of these components.

The composition of the oil will be determined by the considerations previously described. Examples of suitable oils which may be employed are given above. The following further examples of oils are given as illustrations of oils for use in emulsion form for reclaiming weathered asphaltic pavements.

For example, I may employ an oil having the following composition:

Nitrogen bases—Not more than about 20% by weight; First acidaffins—Not more than about 20% by weight; Paraffins—From about 20% to 85% by weight; Second acidaffins—Balance to make up 100%.

Another example of a suitable oil is one containing: Nitrogen bases—Not more than about 35% by weight; Paraffinic fractions—From about 20% to 85% by weight; First and second acidaffins—Balance to make up 100% by weight.

Another example of a suitable oil is one having: Nitrogen bases and first acidaffins—Not more than about 35% by weight; Paraffinic and second acidaffins—Balance to make up 100% by weight;

provided that the paraffinic fraction is in the range of about 20% to 85% by weight of the oil.

Another example of a suitable oil is one containing: Nitrogen bases and first acidaffins—Not more than 20% by weight;

Paraffins and second acidaffins—More than 80% by weight, the total forming 100%, provided the paraffinic fraction is within the range of 20% to 80% by weight.

Other suitable oils are as follows:

TABLE IX

|    |                                          |       |      |       |      |      |
|----|------------------------------------------|-------|------|-------|------|------|
| 60 | Specific Gravity, 60° F./60° F.          | 1.015 | .997 | 1.028 | .966 | .957 |
|    | Viscosity cP at 90° C.                   | 29.9  | 12.7 | 171   | 47.2 | 16.3 |
|    | Initial Boiling Pt., °C.                 | 375   | 360  | 432   | 432  | 380  |
|    | Asphaltenes                              | 0     | 0    | 0     | 0    | 0    |
|    | Paraffins (P)                            | 11.4  | 11.9 | 7.6   | 35.7 | 40.7 |
|    | Second Acidaffins (A <sub>2</sub> )      | 52.9  | 61.4 | 40.7  | 35.4 | 37.2 |
|    | Ratio N+A <sub>1</sub> /P+A <sub>2</sub> | .55   | .36  | 1.1   | .41  | .28  |

<sup>1</sup> At atmospheric pressure.

As a convenient rule of thumb, the boiling point at atmospheric pressure may be assumed to be 140° C. above that at 10 mm. (Hg) pressure absolute.

The  $R_0$  value of the oil may thus range from about 0.01 to about 10, the ratio  $R_0$  chosen depending on the ratio of the asphalt to be improved and on the ratio sought to be obtained. The ratio of the oil to the asphalt will depend on the penetration grade of the asphalt to be improved and the penetration of the improved asphalt

which is desired. Thus, if  $R_a$  of the asphalt to be improved is known, and  $R$  is chosen, and the ratio  $Z$  is established, the equation:

$$Z = \frac{(P + A_2)(R_a - R)}{(P' + A'_2)(R - R_0)}$$

will establish the  $R_0$  of the oil which may be used.

The addition of the maltenes to the asphalt will reduce the penetration of the asphalt, and thus the ratio  $Z$  is dependent on the penetration of the asphalt and on the penetration desired for the improved asphalt.

In the usual case, this ratio  $Z$  will be such as to establish the required penetration grade, to wit, usually, for paving asphalts, in the 85-100 grade or 200-300 grade. However, where special asphalts are desired, other penetrations may be required, and the value of  $Z$  is suitably adjusted.

A further observation is that, if the asphalt to be improved has a ratio  $R_a$  in excess of .4, the value of  $R_0$  is taken as less than  $R_a$ ; and if the value of  $R_a$  be less than .4, the value of  $R_0$  should be greater than  $R_a$ .

If the pavement is badly weathered and cracked, the emulsion will penetrate to the region of weather damage and rejuvenate the weathered asphalt portion of the asphaltic structure.

5 The preferred practice is to use an amount of emulsion of the above concentration, i.e., about 40% oil phase, in at least an amount per square yard which the road will absorb in about fifteen minutes. In cases where early resumption of traffic is not a requirement, larger amounts may be used.

10 This phenomenon is not entirely a viscosity effect, although viscosity does affect the penetration through the pores of the structure. The viscosity of the emulsion, which is substantially that of water, does not control the absorption of the maltenes from the emulsion phase by the asphalt phase of the structure.

15 The following Table X illustrates the effect of the emulsion type on the absorption of the maltenes into the asphalt as it enters the asphaltic structure. It also shows the difference in the effect of other fluids, as named in 20 column 2 of the table.

TABLE X

| Test No.        | Treating Fluid                     |                 | Time of penetration for 10 ml. of treating fluid | Depth of penetration of treating fluid in inches | Time for permeation of 10 ml. Aerosol OT solution into treated briquet |
|-----------------|------------------------------------|-----------------|--------------------------------------------------|--------------------------------------------------|------------------------------------------------------------------------|
|                 | Description                        | Viscosity in cP |                                                  |                                                  |                                                                        |
| 1               | Control                            |                 |                                                  |                                                  | 12 sec.                                                                |
| 2               | Cationic oil emulsion, cone        | 71              | 4 min. 35 sec.                                   | 0.89                                             | 18 min.                                                                |
| 3               | Cationic oil emulsion, diluted 2:1 | 13              | 45 sec.                                          | 0.88                                             | 16 min.                                                                |
| 4               | Cationic oil emulsion, diluted 1:1 | 10              | 30 sec.                                          | 0.89                                             | 18 min.                                                                |
| 5 <sup>1</sup>  | Anionic oil emulsion, diluted 2:1  | 10              | 2 min. 8 sec.                                    | Ran through briquet and out bottom.              | 19 min.                                                                |
| 6 <sup>1</sup>  | Nonionic oil emulsion diluted 2:1  | 12              | 51 sec.                                          | 0.90                                             | 22 min.                                                                |
| 7 <sup>1</sup>  | SS-1 asphalt emulsion, diluted 2:1 | 13              | Dried at surface forming membrane.               | None                                             | 48 min.                                                                |
| 8 <sup>1</sup>  | MC-70 cutback asphalt              | 1,620           | (2)                                              | 0.45                                             |                                                                        |
| 9               | Straight oil                       | 2,660           | 24 hrs.                                          | 0.83                                             | 8 min.                                                                 |
| 10              | Kerosene                           | 5               | 32 sec.                                          | 0.97                                             | 2 min.                                                                 |
| 11 <sup>1</sup> | Oil in kerosene                    | 13              | 2 min. 3 sec.                                    | 0.84                                             | 4 min.                                                                 |
| 12              | Tap water                          | 1               | 16 hrs.                                          | Not measurable                                   | 21 sec.                                                                |

<sup>1</sup> Treating fluid in these tests have same diluent concentration.

<sup>2</sup> Briquet collapsed after 11 to 12 hrs., before complete penetration of fluid.

In treating roads or other asphaltic structures, it is desirable to employ the maltenes in an emulsion form, as will be described below.

The significant importance of an emulsion form of a reclaiming agent for weathered asphaltic pavement arises from the effect of the emulsifier to condition the asphaltic structure and the asphalt phase of the structure, as well as the oil phase of the emulsion, to permit the incorporation of the maltenes phase into the asphalt.

Two different phenomena are to be distinguished. One is the flow of the emulsion fluid through the pores of the asphaltic concrete, i.e., the voids between the aggregate particles bonded by the asphalt, and the other the absorption of the maltenes phase from the emulsion into the asphalt phase to change the chemical composition of the asphalt.

One of the controlling factors is that the emulsion penetrates the surface of the asphaltic structure and passes into the pores of the asphaltic structure but not through the structure before the emulsified maltenes are stripped by the asphalt from the emulsion.

In treating road surfaces for purposes of economy, it is desired to treat the top weathered surface so that its plasticity may be restored. The surface, on rolling either by rollers or by traffic, is thus ironed out and cracks sealed. This preserves the underneath structure. It is undesirable and wasteful to use a treatment which either makes a superficial glaze or runs through the road structure from top to the base. Usually it is sufficient to rejuvenate about the first  $\frac{1}{4}$  to 1 inch of the road surface. This effectively rejuvenates the road and does not waste the emulsion.

45 The specimens used in the tests summarized in Table X were molded briquets, 2.5 inches in diameter, 1.6 inches high, with a 2-inch diameter, 0.318-inch deep reservoir pressed into the top side. The mixture used to form the briquets consisted of 90 parts by weight of 20-30 mesh Ottawa sand (ASTM C-109), 10 parts Portland cement, and 7.5 parts asphalt of 48-penetration.

50 The cationic emulsion was formed using the cationic and nonionic emulsifiers as described above. (See Table X.) The nonionic emulsions were formed using only the nonionic emulsifier (.8% by weight). The anionic emulsions were formed using only anionic emulsifier (1.2% by weight of a sodium petroleum sulfonate).

55 The test procedure employed was to place the test fluid in the reservoir on the top of the briquet and to split the briquet after 24 hours, to determine the depth of penetration by inspection under ultra-violet light. The portions of the briquet reached by the treating agent fluoresce when illuminated with ultra-violet light.

60 It is evident from the test results reported in Table X that a relatively rapid rate of penetration was obtained with all forms of emulsion systems, except the asphalt emulsion (grade SS-1, diluted 2:1 with water), which did not penetrate but formed an asphalt skin at the surface when the water phase evaporated. This notwithstanding that the asphalt emulsion had the same viscosity as the oil emulsions. Further, the anionic emulsion penetrated so easily that it ran through the briquet, and thus the contained oil was not utilized. This is in contradistinction to the cationic and nonionic emulsions.

65 The fact that viscosity is of minor consequence for penetration may further be seen by comparing 11 with

3, in that both fluids had the same viscosity and depth of penetration, but the kerosene-oil mixture penetrated much more slowly.

The oils or cut-back asphalts which are not diluted but are used directly are also not suitable in such form for rejuvenating of weathered roads, since their penetration into the asphalt structure is limited. The same may be said of asphalt emulsion. At best they act merely as a surface coating in the form of a paint. This is illustrated by 7 and 9.

For purposes of comparison, results are also given for kerosene by itself MC-70 liquid asphalt cutback, and tap water.

It is interesting to note that the briquets were relatively impervious to plain tap water but that, with the wetting agent added, water penetrated the briquets readily. The water with the wetting agent even penetrated the briquets that were treated, but at a much slower rate. This serves as a measure of the relative effect on pavement permeability of the various listed treatments, as shown in the last column in Table X.

The duplicate briquets, each separately treated as in the above series, were weathered for 7 days as for the Pellet Abrasion Test. The test method employed consisted of placing the 10 milliliters of the Aerosol OT solution (dioctyl ester of sodium sulfo succinic acid) into the reservoir on top of the briquet and measuring the time for the penetration of the liquid into the briquet. The results reported in Table X show that all emulsion systems tested are more effective in decreasing the permeability of a weathered asphalt-aggregate mixture to the water containing the OT surfactant than are the kerosene cutbacks. Moreover, although the SS-1 asphalt emulsion formed a membrane, water still managed to permeate the structure.

Control 1 is untreated. The permeability of the briquet to the fluid is evidenced by the time of penetration of the fluid through the briquet. Thus, for the untreated briquet (1) the penetration time was 12 seconds, using the aerosol OT water solution. The briquet "treated" with water required 21 seconds. The time for the weathered asphalt treated with the oil emulsions varied from 16 to 22 seconds, that for the nonionic emulsions being slower than the cationic emulsion containing also the nonionic emulsifier.

In addition to the tests reported in Table X, a number of other fluids were tested to check on the importance of the emulsification system. One of these tests was the use of a straight cationic emulsion, i.e., an emulsion the same as used in test 3 but *not* containing a nonionic emulsifier, only the cationic. The viscosity was substantially the same (14 centipoises), but the time of penetration for 10 ml. of the treating fluid into the briquet was 162 seconds. The depth of penetration was 0.81 inch. The time of permeation of 10 ml. of Aerosol OT solution in the aged treated briquet was 21 minutes. A comparison of these figures with those shown in Table X for test 3

demonstrates the difference between a cationic-nonionic emulsification system and a straight cationic. Depth of penetration was slightly less for the straight cationic system, but the time of penetration was about 3 times that of the nonionic-cationic system. The slower permeation of the Aerosol OT solution into the briquet treated with the straight cationic emulsion can be explained by the more efficient stripping of the maltenes from the emulsion by the asphalt, as evidenced by the lower depth of penetration into the briquet and thus increased density of the treated portion of the briquet.

The above data is further evidenced that the effect of the oil emulsion on asphaltic concrete is not a viscosity effect, but is strongly affected by the nature of the systems, the oil emulsion system showing a markedly different and more rapid penetration than do other systems of similar viscosity, resulting in less permeable structures.

This effect is further demonstrated by actual field test experience. A weathered road was treated with a cationic emulsion containing additionally a nonionic emulsifier similar to that employed in the tests shown in Table X.

A weathered asphaltic road was treated in sections with a 2:1 dilution of a cationic maltenes emulsion containing nonionic emulsifier, such as described in connection with Table X, employing 0.06 gallon/square yard, 0.14 gallon per square yard, and an excess quantity, approximately 0.25 gallon per square yard. Another section was treated with conventional asphalt emulsion SS-1h (slow setting emulsion containing 60 penetration asphalt), with a dilution of approximately 3:2 at the rate of 0.1 gallon per square yard. A section was left untreated.

From visual observations during application, it was evident that the diluted maltenes emulsion penetrated into the five-year-old pavement quite readily, with complete penetration being accomplished within five to twenty minutes, depending on the rate of spread. Since this pavement had not previously been sealed, and since there were no accumulations of grease drippings, no sanding was required. On the other hand, the asphalt emulsion did not penetrate, and sanding was required for safety reasons and to prevent pick-up of the asphalt by traffic.

Two months after application, cores were taken from the various sections and cut horizontally at  $\frac{1}{2}$ -inch intervals. Viscosities of the asphalt recovered from each slice were then determined using the sliding plate microviscometer, manufactured by Hallikainen Instruments, Berkeley, California. See articles by Labout and Van Ort in Anal. Chem., vol. 28, 1147-1151 (1956) and Griffen et al., in Road and Paving Materials (A.S.T.M.) Special Technical Publication 212 (1957), pages 36-50. Table XI is a tabulation of the viscosities measured and the penetration (given in parentheses) derived from the viscosities. (See Pfeiffer, "The Properties of Asphaltic Bitumens," published by Elsevier, New York, 1950, p. 160.)

TABLE XI  
*Viscosity of Recovered Asphalt, Megapoises*

| Depth, In.                       | Untreated | Cationic Maltenes Emulsion, diluted 2:1 |            |                    | Asphalt Emulsion |
|----------------------------------|-----------|-----------------------------------------|------------|--------------------|------------------|
|                                  |           | 0.06 gsy                                | 0.14 gsy   | 0.25 gsy (approx.) |                  |
| 0- $\frac{3}{8}$                 | 86 (12)   | 7 (36)                                  | 0.35 (148) | 0.2 (185)          | 45 (15)          |
| $\frac{1}{2}$ - $\frac{3}{8}$    | 21 (21)   | 19 (22)                                 | 11.4 (29)  | 6.3 (38)           | 16 (24)          |
| 1- $\frac{1}{8}$                 | 19 (22)   | 15 (25)                                 | 10.5 (31)  | 8 (34)             | 15 (25)          |
| 1 $\frac{1}{2}$ -1 $\frac{1}{8}$ |           |                                         |            | 11 (29)            |                  |

NOTE.—Numbers in parenthesis are penetration values of asphalts obtained by conversion. See text.

It is quite apparent from Table XI that the treatment with the maltenes emulsion has caused a significant change in asphalt viscosity present in the pavement to a depth of at least  $\frac{1}{2}$  inch, with a possible effect of the added maltenes to a depth of  $1\frac{1}{4}$  inches of the heavier treatments. Since these results were from cores taken relatively soon after application (approximately two months), it is possible that the maltenes had not yet had sufficient time to reach a state of equilibrium with the asphalt. In the case of the asphalt emulsion of substantially the same viscosity, no such effect is observed.

The cationic emulsion of the maltenes produces asphaltic structures of improved cohesiveness as compared to other dilution systems. They have improved load-penetration characteristics. Tests were run on the same type of briquet used in comparing rates and depths of liquid-penetration. (See Table X.) An apparatus was used which would apply load to the treated end of the briquet through a 1.128-in. diameter (1.0 sq. in.) piston at a strain rate of 0.25-in. per minute to a total deformation of 0.250-in. The data obtained from this test are relative but valid for the series of briquets tested. Resulting load vs. deformation diagrams were obtained and are shown in FIG. 5.

In order to establish reference points on the chart, two load-deformation curves are shown for freshly mixed briquets made with 7½ percent by weight of 48 penetration and 200-300 penetration asphalts. All other curves represent various treatments of a reference briquet made with 48 penetration asphalt at various states of aging. The aging of the briquets was accomplished in the infrared oven described in the article by Rostler and White, *supra*. The oven is automatically controlled so that the temperature within the briquets themselves is maintained at 140° F. during the specified aging time.

From FIG. 5 it is evident that kerosene used as a carrier destroys the cohesiveness of asphalt binder and that proper cohesion cannot be regained even after 14 days of exposure at 140° F. in the infra-red oven because the kerosene has dislocated that asphalt cement located between the points of aggregate contact. In contrast, the emulsion system used for introducing the maltenes does not displace the asphalt providing the bonds between aggregate particles in the briquets, as evidenced by the fact that in all cases the briquets have resistance to load penetration exceeding that of 200-300 penetration asphalt, although the consistency of the binder (asphalt) has been lowered.

From laboratory studies similar to those described above and from field experience in applying various emulsions to pavements, it has been concluded that the best method for incorporating the maltenes into the weathered asphalt concrete, as in road pavement, is in the form of a fine particle size, cationic emulsion, containing a nonionic emulsifier, as described. Although a dilution rate of two parts of emulsion concentrate to one part of water (40% oil content) is preferred to get the best combination of penetration rate and economy, the dilution rate to fit each particular job should be chosen on the basis of job conditions.

The importance of the emulsion system as affecting the particle charge is shown by the following.

One series of tests was designed to determine the importance of particle charge, as related to the adhesion characteristics of the asphalt-aggregate system. The test consisted of placing 2-g. pellets made by mixing 100 parts Ottawa sand and two parts 85-100 penetration asphalt, aged for seven days in the infra-red oven at 140° F., into beakers containing 50 ml. distilled water and heating the water to the boiling point. For this test several pellets were prepared and tested after treatment with 0.06-g. of the maltenes. The oil was applied as a cationic-nonionic emulsion, described above, and as a nonionic emulsion, undiluted, and as a solution in kerosene. The pellets, after aging for seven days in the infra-red oven at 140°

F., were immersed in 50 milliliters of water, the water heated to boiling, and the contents of the beaker filtered through a No. 1 Whatman filter paper. The stripping effect was evaluated by observing the amount of asphalt floating at the water surface and clinging to the beaker walls, as well as by noting the area of exposed aggregate surfaces on the Ottawa sand at the bottom of the beaker.

The relative effect of the test on stripping of the asphalt could be readily observed visually. Most of the asphalt was stripped off the sand grains in the untreated control pellet and all of the other treated pellets, except the one treated with the cationic emulsion of the maltenes, where very little stripping was noted. The stripping that was observed in the cationic sample was due to asphalt stripped from the bottom of the pellet where the treatment did not reach.

Another test consisted in examining under a microscope fragments of the treated pellets in order to observe the effect of the treatment and aging procedure on the asphalt cementing the sand grains in the pellets. Improvement in the bonding accomplished by the cationic emulsification system, which causes the oil to wet preferentially the asphalt portion of the asphalt-sand mixture, was readily observable.

This microscopic examination showed that the nonionic emulsion system does little to increase the bond because there is no preferential wetting of the asphalt portion. The undiluted maltenes result in droplets of uncombined oily material attached to the sand grains.

With kerosene as a carrier for the oil, the asphalt films are washed from the sand grains and are accumulated in the voids between them, resulting in loss of bond at the points of contact.

The advantageous results obtained from using the above combination of emulsifiers is additionally shown in the following tests.

Abrasion tests pellets were prepared in accordance with the Pellet Test procedure referred to above, using a 48-penetration asphalt and 20-30 mesh Ottawa sand. Duplicate pellets without treatment, and also duplicate pellets treated with aqueous emulsions of the maltenes in the same concentration of maltenes but differing only in the emulsion system, were subjected to the following tests. The cationic emulsion was that previously described containing nonionic emulsifier. The nonionic emulsion was made from the nonionic emulsifier alone, and the anionic emulsion contained only an anionic emulsifier. The pellets were then aged in the infra-red cabinet for seven days (see Rostler and White, *supra*).

After exposure in the infra-red oven employed in the above procedure, the weathered pellets were subjected to an abrasion test by tumbling them in a 16-oz. French square bottle for 500 revolutions, as in the above Pellet Test.

Table XII summarizes the results obtained in this abrasion test.

TABLE XII

| Pellet Abrasion Test Results |                                                                      |
|------------------------------|----------------------------------------------------------------------|
| Treatment:                   | Abrasion Loss, Percent (average of duplicate specimens), 7-day Aging |
| Untreated Control            | 34                                                                   |
| Cationic Emulsion            | 13                                                                   |
| Nonionic Emulsion            | 19                                                                   |
| Anionic Emulsion             | 21                                                                   |

It will be seen from the above results that the cationic emulsion showed a considerably greater improvement in the abrasion loss after 7 days as compared with the other emulsion systems, the cationic emulsion showing a 62% reduction, the nonionic emulsion a 44% reduction, and the anionic emulsion a 35% reduction in the abrasion loss.

The effect of the maltenes in the cationic-nonionic emulsion form in modifying the asphaltic phase of an asphaltic pavement is further illustrated by Table XIII, showing the effect of this treatment on the permeability of the road pavement to water.

The emulsion is stable in the sense that it will not break when stored for long periods in clean, closed containers at ordinary atmospheric temperature above freezing. Additional water may be introduced into the emulsion prior to time of application.

TABLE XIII

|                                                                                                                                         | Station    | Water Permeability, Mls./Min. |     |     |
|-----------------------------------------------------------------------------------------------------------------------------------------|------------|-------------------------------|-----|-----|
|                                                                                                                                         |            | OWT                           | BWT | IWT |
| Test Section: Section treated with cationic-nonionic-maltenes emulsion. Rolling same as control section. Section 1.                     | A          |                               |     | 45  |
|                                                                                                                                         | B          |                               | 40  |     |
|                                                                                                                                         | C          | 50                            |     |     |
|                                                                                                                                         | D          |                               |     | 25  |
|                                                                                                                                         | E          |                               | 40  |     |
|                                                                                                                                         | F          | 40                            |     |     |
|                                                                                                                                         | G          |                               |     | 28  |
|                                                                                                                                         | H          |                               | 135 |     |
|                                                                                                                                         | I          | 30                            |     |     |
|                                                                                                                                         | J          |                               |     | 47  |
|                                                                                                                                         | K          |                               | 90  |     |
|                                                                                                                                         | L          | 80                            |     |     |
|                                                                                                                                         | M          |                               |     | 40  |
|                                                                                                                                         | Ave.       | 50                            | 76  | 37  |
|                                                                                                                                         | Total Ave. |                               | 54  |     |
| Control Section: Rolling consisted of breakdown with 12 T tandem + 3 coverages with 26 T pneumatic followed with 8 T tandem. Section 2. | N          |                               | 135 |     |
|                                                                                                                                         | O          | 85                            |     |     |
|                                                                                                                                         | P          |                               |     | 75  |
|                                                                                                                                         | Q          |                               | 105 |     |
|                                                                                                                                         | R          | 100                           |     |     |
|                                                                                                                                         | S          |                               |     | 77  |
|                                                                                                                                         | T          |                               | 180 |     |
|                                                                                                                                         | U          | 120                           |     |     |
|                                                                                                                                         | V          |                               |     | 40  |
|                                                                                                                                         | W          |                               | 190 |     |
|                                                                                                                                         | X          | 65                            |     |     |
|                                                                                                                                         | Y          |                               |     | 60  |
|                                                                                                                                         | Ave.       | 93                            | 153 | 61  |
|                                                                                                                                         | Total Ave. |                               | 102 |     |

OWT=outer wheel tracks.

BWT=between wheel tracks.

IWT=inner wheel tracks.

Tests were made by treating a road to ascertain the effect of the emulsion on the water permeability of a newly compacted asphalt pavement. In Table XIII are given water permeability results from tests conducted on the pavement immediately after final compaction. All water permeability tests were run on the surface course using the method described in California Test Method 341-A.

As seen in Table XIII, the test section with the maltenes emulsion treatment has had its water permeability reduced to about 53 percent of the untreated control section. This is an extremely important feature of the maltenes emulsion treatment, particularly when one considers the compaction effort required to reduce the permeability to a similar degree. Moreover, the decrease in permeability has been achieved in a finite depth of the pavement, and not by a skin coating which can readily be worn away by weather and traffic.

The superiority of the balanced emulsions containing the blend of the cationic emulsifier and the nonionic emulsifier, as shown by the above tests, is confirmed by actual field experience.

These cationic emulsions have the additional superiority that they are stable and may be mixed with hard water and even sea water without breaking the emulsion.

I have found that, for the purposes of my invention, the emulsion should preferably have the following characteristics: It should be free-flowing, preferably within the range of 57 to 63 parts of the oily component by weight, and water as the continuous phase not less than about 25 parts by weight and preferably in the range of 37 to 43 parts by weight, and also an emulsifier. Water employed may be distilled water, or ordinary soft or hard waters.

I have found that the best results are obtained by using a balanced type emulsion, as described above. The emulsifiers to be employed are preferably surfactants which are stable under the conditions employed in making the emulsion, and which will not break immediately when applied to the road or other asphaltic structure being reclaimed, so as to penetrate the asphalt and release the oil phase, i.e., the maltenes, within the asphalt structure, to become incorporated into the weathered asphalt.

The surfactant compounds having properties previously described are listed in standard textbooks in this art, for example, the Encyclopedia of Surface Active Agents, by Sisley and Wood, published by the Chemical Publishing Company, Inc., New York. The cationic emulsifying agents employed may be, for example, Cetylpyridinium chloride, or other quaternary ammonium salts and other cationic surfactants listed in the above publication and other standard books on the subject. These include the aliphatic fatty amines and their derivatives, the homologues of the aromatic amines having fatty chains (see pages 35, etc., 95-105, of the 1952 edition of the above publication). Nonionic emulsifying agents such as are described above, and others which have the properties previously described, may be employed, such as are listed in the above text book, at pages 119-123 and page 163, etc.

Suitable nonionic emulsifiers which have been employed are nonionic surfactant sold by Process Chemical Company as Pronon 280, and as Oronite NI-W by the Oronite Chemical Company, and believed to be dodecyl phenol polyethoxyethanol. Suitable cationic emulsifiers are the fatty quaternary ammonium salts, fatty amido-amino-amine salts of the lower fatty acids sold by Process Chemical Company as Promine 2118, and believed to be a fatty

amido-aminoamine acetate, and also the propionate salt sold as Promine 2115.

This list is not intended to be exhaustive, and is but suggestive of the emulsifying agents which may be employed. Many agents useful for emulsifying petroleum oils are effective in various concentrations.

In addition to the emulsifying agent, stabilizers may be used to stabilize the emulsion against electrolytes which may be present in the water used for making or diluting the emulsion.

The emulsion has the surprising result discussed above, in that it causes a rapid penetration of the reclaiming agent into the weathered structure, such as a weathered road. The rate of penetration depends also on the porosity of the road. This depends on the density, i.e., the compaction of the road when laid down, the grading of the aggregate, the original asphalt content of the road and the degree of weathering. Depending on these factors, the emulsified maltenes of my invention will be absorbed from almost instantaneously up to about 2 days, depending upon the volume per unit area of road. Unemulsified maltenes applied in equivalent volume rate calculated as oil, on a like road surface, will, experience has shown, take from several hours to a week or more, and in some cases will not be absorbed at all. During all this period the road is slick and unsafe for traffic.

Highway regulations in California require two lanes to be opened by sun-down, and for many roads this is not possible, using unemulsified oil; whereas with an emulsion used according to my invention, such penetration is achieved.

When using an emulsion made with a nonionic emulsification system on processed roads which had a large amount of dirt and dust incorporated by the breaking up process, the emulsion appeared to preferentially wet the unoiled aggregate and dirt and acted as a dust-layer and did not penetrate the asphalt very well. When the emulsion is made with a cationic emulsifier, the weathered asphalt-coated surfaces are preferentially wetted, but a mixed cationic-nonionic emulsification system is preferred because it provides a balance of desirable properties, to wit: ease of emulsification; stability in storage and application; rapid penetration; preferential wetting of asphalt rather than of aggregate; and a water-repellent surface on the reclaimed structure.

I have found that materially improved results may be obtained by employing a balanced emulsion. By a balanced emulsion I mean an oil and water emulsion stable against electrolytes present in hard water and containing nonionic surfactants and cationic surfactants in amounts sufficient to form an emulsion of cationic character, i.e., one in which the oil phase will deposit on the negative electrode if the emulsion is subjected to electrophoresis. Thus, the preferred emulsion will contain in parts by weight, based upon the oil phase of the emulsion, nonionic surfactants from 0.5% to 2% and cationic surfactants from 0.5% to 1.5%. Preferably the surfactant should be employed in the emulsion in an amount, based upon the oil phase, such that the nonionic surfactants are preferably about 0.7% or more by weight and cationic surfactants of 0.5% or more. Such an emulsion system will wet the asphalt portion of the road surface preferentially over the wetting of the aggregate and penetrate into the capillaries of the wetted asphalt at a more rapid rate than if no nonionic surfactant were employed.

For the purpose of convenience, I prepare the emulsion in the above concentrations. Before applying the emulsion to the road, I may dilute the emulsion, for example, with an equal amount of water, although higher or lower dilutions may be employed.

The amount of maltenes to be added to the weathered asphalt depends on the nature of the weathered asphalt. In the case of an asphaltic pavement, the amount of the maltenes to be added should be not so great as to make

the pavement unstable and should not exceed the safe asphalt content of the road, nor be used in an amount such as to cause syneresis, i.e., oil exudation. Additionally, the amounts added should be sufficient to improve the quality of the road or other asphaltic structure above that of the weathered road or structure, but not in such large quantity as to exceed, in the case of a road or other asphaltic structure, the capacity of the road or other structure to absorb the fluid applied, as will be described below. The amount of the total asphalt should not exceed the safe holding power of the aggregate. If it is exceeded, the asphalt will exude as a separate phase and not be incorporated into the asphaltic structure. Various authorities specify the particular composition of asphalt pavement, and thus determine the quantity of asphalt to be contained in the asphalt pavement.

Standard Specifications issued by the Division of Highways, Department of Public Works, State of California, dated August 1954, gives at page 321, etc., the properties of various asphalts which were acceptable to the State of California. See also "Asphalts and Allied Substances," by Abraham, 5th Ed., vol. 1, page 643, published by D. Van Nostrand & Co. The particular penetration grade asphalt found acceptable for any specific road job is usually specified by the engineer on the job or by contract. Thus, the required penetration grade for a good structure acceptable to the owner may be determined.

The concentration and amount of emulsion to be applied to the road surface is further controlled by the requirement that the emulsion be absorbed into the road surface without wasteful run-off. The quantity of emulsion to be employed on the road depends thus also on the permeability of the road. Road permeability, measured as milliliters of water absorbed per minute by the road, may be determined by the test procedure California 341-A, issued January 1960, by the Materials and Research Department, Division of Highways, Department of Public Works, State of California. To determine the rate of application of the emulsion to the road in treating either freshly laid or weathered roads, the following modification of the above California 341-A procedure, known as the grease ring test, may be used.

The above emulsion concentrate, diluted with half its volume of water, is applied to the road within the six-inch diameter grease ring, formed as described in California Test 341-A. The time to absorb measured incremental volumes of the diluted emulsion is measured. This is continued until, as in the California test, the surface remains wetted after prolonged standing. From this data the volume applied per square yard of the top surface of the road, required to be absorbed in a given time, e.g., 15 minutes, is determined.

In addition to rejuvenating weathered asphaltic roads, it has been found that the treatment also acts as a "seal in depth." After penetrating into an asphalt pavement, it combines with and expands the asphalt. Permeability of the pavement to water is reduced. In some instances, where initial shrinkage cracks had developed, the treatment reverses the shrinkage process and closes the cracks. Moreover, when placed between successive layers of asphalt pavement, it provides an excellent bond by promoting a fusing of the asphalt layers at the interface.

Because of its ability to act as an asphalt replasticizer, as a "seal in depth" and as a bonding agent, the maltenes emulsion described can be used on all types of asphalt paved surfaces not only in preventive and corrective maintenance but also in construction and reconstruction operations.

In preventive maintenance, the emulsion is applied to a structurally sound asphalt pavement as soon as it begins to show signs of aging or brittleness through the symptoms of dryness, surface pitting, ravelling or shrinkage cracking. Generally, these conditions develop in a period of two to ten years after construction, de-

pending on such factors as mix design, asphalt durability, pavement permeability and climatic conditions. Here the abject is to penetrate the asphalt pavement and re-plasticize the asphalt before deterioration of the pavement due to brittleness has progressed too far.

Pavements that have developed a traffic "glaze" from high density traffic and grease drippings sometimes require removal of this seal to facilitate penetration.

In corrective maintenance, the oil emulsion is used in conjunction with other procedures to improve an asphalt pavement which is structurally sound but is extensively pitted or badly cracked. Usually the surface requiring treatment must be scraped or loosened in some convenient way and the loose material discarded or sprayed and recompacted. It may also be desirable to incorporate a new mixture of sand and asphalt in the loosened treated surface, in order to provide a proper balance of aggregate and asphalt.

In reconstruction, the oil emulsion may be used to re-plasticize existing asphalt paved surfaces prior to a resurfacing operation or as an aid in breaking up and reworking an old, weathered asphalt paving while simultaneously re-plasticizing the asphalt in the mix. In the latter case, the treatment may be sufficiently effective to make the mix reusable again as a surface course.

In new construction the treatment, which is applied after the asphalt paving has been spread and compacted, serves two purposes. The maltenes penetrate the surface and combine with the asphalt to restore the properties lost in the mixing cycle at the hot plant. The maltenes also combine with the asphalt to cause the asphalt to expand and close the pores of the pavement, thereby sealing the pavement to the depth of penetration of the oil.

By far the simplest method of bringing together the maltenes and the aged asphalt is by spraying a predetermined quantity of emulsion on the pavement surface and allowing it to soak in. This procedure is always effective in preventive maintenance, in new construction seals and in priming and tack coating operations. Conventional calibrated asphalt spreader trucks may be used.

It has been found that all newly laid asphalt paving and the majority of weathered asphalt pavements, whether asphalt concrete, plant mix or road mix, are sufficiently permeable to respond to this simple "spray and penetrate" approach, provided a seal coat has not previously been applied. The "grease ring" test described above provides a method for determining the amount of the emulsion to be applied in one operation.

If the pavement has had a so-called asphalt emulsion "fog" seal, there is usually no difficulty in getting penetration, as this type of seal weathers rapidly and wears off in a short time. However, the "fog" seal does present a problem calling for special precautions, as the weathered remnants of the "fog" seal will combine with and hold a certain amount of maltenes at the surface, causing a slippery condition. In such instances, a light sanding is necessary, about 1 to 2 pounds of fine, dry sand per square yard, before traffic can be allowed on the pavement. It is preferable, however, that sanding not be done before the emulsion has had at least 15 minutes and preferably 45 minutes to penetrate into the pavement.

The following examples illustrate the use of the emulsions for pavements in various stages of distress requiring treatments ranging from preventive maintenance to complete reconstruction.

#### EXAMPLE 1

The California Standard Specifications previously described give the quantity of asphalt to be applied to a road structure. Examples taken from the California Standard Specifications will illustrate this.

Thus, at page 143, for Asphalt Concrete Pavement the requirement is:

|   | Course—Asphalt percent based on total mix: | Percent |
|---|--------------------------------------------|---------|
| 5 | Base                                       | 4-5.5   |
|   | Leveling                                   | 4-5.5   |
|   | Surface                                    | 4-6     |

I may add sufficient maltenes to bring the total of asphalt, including the added fraction, based on the sample extracted, up to about the maximum percentage permitted by the specification for the road; thus, 6% for the specifications given above. I may, however, exceed this maximum percentage allowed by such specifications by about 2%, increasing the asphalt content to about 8% instead of 6%, i.e., increase the asphalt content to about 1.2 to about 1.3 times the specification requirement, particularly when determining the desirable asphalt content to be established in reclaiming, in place, a weathered road or asphalt pavement.

Reference may also be had to the manual on "Design and Construction of Asphalt Roads and Streets," issued by the Asphalt Institute Pacific Coast Division, page 66, Section H(6e), 1952 Edition, for methods of determining the allowable percentage of asphalt to be present in various asphalt structures.

The formula for the percentage by weight of asphalt to be used in the mixture with the aggregate, in producing a fresh asphaltic pavement mix from asphalt and aggregate, is given by the formula:

$$P = (R \times 4 + S \times 7 + F \times 12)C$$

Where

$P$ =the percentage by weight of asphalt to be used in the mixture with the aggregate;

$R$ =the decimal percentage of rock in the mix;

$S$ =the decimal percentage of sand in the mix;

$F$ =the decimal percentage of silt in the mix;

$C$ =circumstantial factor, which normally is 1.

In order to determine the amount of maltenes to be added, according to the procedures of this invention, I may proceed in the following manner.

A core taken from the weathered road was treated to extract the asphaltic content of the road, and the extract asphalt determined by the method previously described on pages 31-32 of this specification.

The sieve analysis of the recovered aggregate is performed according to the above Asphalt Institute reference. Due to the fact that the weathered asphalt partakes somewhat of the nature of an oxidized asphalt, I have found that the reclaimed road will tolerate an amount of asphalt up to about 30% in excess of the amount specified according to the above formula, i.e., to a value equal to about  $P + .3P$ . Knowing the weight of the asphalt in the core as determined above, and the top surface area of the core, the weight of the maltenes in emulsified form to be added per square yard of the surface of the road may be readily calculated.

Since the addition of maltenes is limited by the amount which the road can tolerate and be stable, i.e., form a homogeneous body without exudation of oil as a separate phase, it has been found that a practical application without a preceding core analysis may be made. This procedure depends on the nature of the surface.

The following examples illustrate the methods applied to the above cases. They are given as illustrations of, and not as limitations of, my invention.

#### EXAMPLE 2

This procedure for relaying completely deteriorated 70 road surfaces consists of three steps:

(1) Breaking up of the road to give pieces exposing sufficient fractured surfaces for the emulsion to penetrate the aged asphalt, e.g., pieces with no dimension substantially over 4 inches.

(2) Spraying the broken-up pieces with  $\frac{1}{4}$  to  $\frac{1}{2}$

gallon of the emulsion per square yard per inch depth. (In most cases dilution of 4 parts of the above emulsion with 1 part of water before application is recommended to reduce the viscosity of the emulsion and thus to facilitate penetration.)

(3) Regrading and compaction—This operation can be carried out with standard road building equipment. If the asphalt to be reclaimed is from an abandoned pavement, then the product after step (2) can be kept in a stock pile for later use.

The machinery used is (1) a grader equipped with scarifier teeth and a blade; (2) a grader equipped with a set of discs and a blade; and (3) a road oil truck equipped with spreader bar and pump to deliver the emulsion in required amounts.

The surface is first broken up by means of the scarifier teeth of the grader, then further broken by the discs of the other grader, set to reach down to the base. The blades are used to turn and mix the broken pieces. After running this equipment back and forth several times to break up the road surface, the surface is leveled by the blade. The spreader truck is then driven over the broken-up surface and a suitable dilution of the emulsion is sprayed on the mix; for example, a 1:1 concentrated emulsion-to-water mix, at the rate of 1½ gallons per square yard. The emulsion quickly penetrates the broken-up material, coating each individual particle of the mix and depositing a film of the emulsion on the base. The treated mass is then mixed back and forth several times by the blade, and is then graded with a blade. The surface is then compacted by the wheels of the graders. (In some cases a properly graded, reworked surface can be left to automobile and truck traffic for compacting.)

Even in cases where the road shows considerable brittleness and large cracks, it often suffices to scarify the road surface slightly, to spread the required amounts of the emulsion onto the surface and let capillary action carry the reclaiming agent into the pavement. If the surface is uneven and badly cracked, it is advisable to fill the cracks with an asphalt-sand mix and to cover the whole road with a thin layer of this mix in order to form an even surface.

#### EXAMPLE 3

Procedure of Example 2 is to be used with asphalts which have deteriorated to a stage of brittleness which needs drastic measures for repairing the damage. Although much more economical and much more effective than other methods of repairing deteriorated asphaltic pavements, this procedure may be considered to be only a salvaging operation. Considerable more economy can be achieved by revitalizing asphalt pavements in a planned preventive maintenance program consisting of regular inspections of roads and corrections of damage due to natural aging at its onset, by application of the emulsion of this invention in the process of this invention.

Preferably the procedure of Example 3 is started as soon as the road is constructed and should take place not later than when the first stage of hardening is evidenced by the appearance of hair cracks. At this stage of the aging process, spraying of the surface with small amounts, for example, 0.05 to 0.15 gallon per square yard per inch depth (sometimes followed with a light application of sand), reverses the aging process and gradually restores the asphalt to its original plasticity. It can be expected that such maintenance, started soon after completion of the road and repeated when needed, will prolong the life of flexible pavements far beyond their original life expectancy. This is the type of operation recommended as preventive maintenance.

Many roads are, however, already in existence and in need of maintenance. Some of the existing roads will be in a condition between the two described under Example 2 and Example 3 and will consequently require maintenance measures between the two methods suggested. This is illustrated by Example 4.

#### EXAMPLE 4

The operation may include scarifying the road surface by means of discs or heater-planers, removing loose dirt, cleaning out larger cracks in the pavement, filling the cracks with repair material (asphalt reclaimed by use of the emulsions described herein, taken from a stock pile, is highly suitable), and spraying the emulsion with a spreader truck onto the surface. The amounts of emulsion to be used are usually between about 0.1 to about 0.2 10 gallon per square yard per inch depth of pavement.

#### EXAMPLE 5

The composition of the emulsion described herein has been designed to be usable for all three procedures of 15 Examples 2-4 and with all asphalts. The difference in degree of aging of different asphalts is taken into account in the recommendation of the amounts of the emulsion to be used. For areas large enough to warrant individual consideration, it is suggested that cores be taken from the 20 pavement, the asphalt extracted and analyzed. From this analytical data a special emulsion and application can be devised.

In designing a revitalizing procedure exactly tailored to fit a particular asphalt, one of the principal precautions to observe is to add the right amount of reclaiming 25 agent, in order not to exceed the total amount of asphalt permissible for the particular mix, i.e., to stay within the stability limits prescribed for the pavement. As shown by laboratory tests and field trials, reclaimed pavements 30 can tolerate (as can constructions made with artificially oxidized—i.e., air blown—asphalt) 20% to 30% more asphalt than aggregate-asphalt mixes made with regular steam reduced asphalts.

The precaution not to exceed the permissible amounts 35 of asphalt in the mix is automatically taken care of, in the procedure of each of the Examples 2-4, by adding in small increments, observing the workability of the mix after each addition, and stopping when the desired degree of plasticity has been obtained. The following example 40 is an illustration of a specially devised application.

A core taken from a weathered road was extracted with benzol by the method previously described. The recovered extract asphalt was analyzed to determine its composition. The silt from the filter was combined with 45 the aggregate from the extraction thimble, dried, and sieved to determine the grading of the aggregate. The extraction gave the following results:

|                                     | Percent by weight of core |
|-------------------------------------|---------------------------|
| Recovered extract asphalt           | 4.6                       |
| Recovered aggregate                 | 94.3                      |
| Loss (water and dust)               | 1.1                       |
| Analysis of recovered asphalt:      |                           |
| Asphaltenes (A)                     | percent 31.3              |
| Nitrogen bases (N)                  | do 28.7                   |
| First acidaffins (A <sub>1</sub> )  | do 10.1                   |
| Second acidaffins (A <sub>2</sub> ) | do 13.1                   |
| Paraffins (P)                       | do 16.8                   |
| N+A <sub>1</sub> /P+A <sub>2</sub>  | 1.3                       |

Sieve analysis of recovered aggregate (according to procedure given in "Design and Construction of Asphalt Roads and Streets," issued by Asphalt Institute, Pacific Coast Division, 1952 Edition, p. 66, Section H (6e)):

|                                                       | Percent |
|-------------------------------------------------------|---------|
| Rock portion, retained on 4 mesh screen               | 68.2    |
| Sand portion, passing 4 mesh and retained on 200 mesh | 26.2    |
| Silt portion, passing 200 mesh screen                 | 5.6     |

The formula for maximum allowable asphalt content given in the above reference is applied as follows:

$$P = [(R \times 4) + (S \times 7) + (F \times 12)]C$$

Where

$P$ =percentage of asphalt to be used;  
 $R$ =decimal percentage of rock;  
 $S$ =decimal percentage of sand;  
 $F$ =decimal percentage of silt;  
 $C$ =circumstantial factor, which has been found to be 1.2 to 1.3 for reclaiming of weathered asphalts;

Thus,

$$P = 1.25[(0.682 \times 4) + (0.262 \times 7) + (0.056 \times 12)] \\ = 1.25(5.23) \\ = 6.54\% \text{ maximum permissible asphalt content.}$$

The difference between this figure and the actual asphalt content of road (6.54-4.6=1.94) represents the amount of reclaiming agent which can be added without loss of stability of the pavements (i.e., bleeding and deformation).

In this particular example only 0.65% reclaiming agent was required to restore the asphalt to approximately its original consistency, so this amount was used. The difference between the maximum and the present asphalt content of the reclaimed road (6.54-5.25=1.29) indicates that it will be possible to reclaim this road again when the need develops, without risking loss of stability of the pavement.

#### EXAMPLE 6

A road which was about four years old has been laid employing an asphalt, a retained sample of which was analyzed by the method previously described.

A core taken from the weathered road was treated to extract the asphaltic content of the road.

The analysis of the extract of the weathered asphalt and the retained sample of the original asphalt is given in the following table:

|                                     | Original Asphalt,<br>percent by weight | Extract Asphalt,<br>percent by weight |    |
|-------------------------------------|----------------------------------------|---------------------------------------|----|
| Asphaltenes                         | 28.0                                   | 40.8                                  | 40 |
| Maltenes:                           |                                        |                                       |    |
| Nitrogen Bases (N)                  | 14.0                                   | 8.0                                   |    |
| First Acidaffins (A <sub>1</sub> )  | 8.5                                    | 7.2                                   |    |
| Second Acidaffins (A <sub>2</sub> ) | 40.4                                   | 35.4                                  |    |
| Total                               | 62.9                                   | 50.6                                  | 45 |
| Paraffins (P)                       | 9.1                                    | 8.6                                   |    |
|                                     | 100.0                                  | 100.0                                 |    |
| N+A <sub>1</sub> /P+A <sub>2</sub>  | 0.46                                   | 0.35                                  |    |

The extract asphalt constituted 4.4% of the weight of the sample.

It will be observed that this asphaltenes content of the asphalt has increased by 12.8%, while the saturated hydrocarbons have been substantially unchanged. The half percent loss of paraffins may be ignored as a combination of error of measurement, or evaporation loss during aging. There has been a substantial decrease in the nitrogen bases and second acidaffins. These products are the source of the increase in the asphaltenes content, and their disappearance has resulted in the deterioration of the asphalt. The  $N+A_1/P+A_2$  ratio of the original asphalt was 0.46, within the preferred range, and on weathering it was reduced below the 0.4, to wit, to 0.35. The weathering process reduced the ratio from Group 1 (see FIG. 1) to group 0, where, according to Table I, are included asphalts whose abrasion resistances are inferior to those of Group 1.

While I do not wish to be bound by any theory of the chemical activity or inactivity of any of the asphaltenes components, I have found that, in order to determine the amount of the maltenes to be added, I may treat the asphaltenes content in excess of the asphaltenes content of the original asphalt as inert and as if it forms part of the silt in the aggregate material in the sample.

The remaining asphaltenes thus correspond to the asphaltenes content of the original asphalt. The loss of

the maltenes components thus has reduced the total quantity of asphalt by 12.8%.

The asphalt is reclaimed by adding maltenes components sufficient to re-establish the balance of the maltenes components to asphaltenes, ignoring the 12.8% as inert aggregate and balancing only as against the original 28% of the asphaltenes.

Thus, by adding 12.8 parts of the maltenes to 100 parts of the extract asphalt (as determined by the extraction previously referred to and by analysis of the extract asphalt as previously) I obtain the following results. Maltenes were added as an emulsion of 60 parts of maltenes to 40 parts of water prepared as described above.

#### 15 Maltenes added:

|                   |         |      |
|-------------------|---------|------|
| Asphaltenes       | Percent | 0    |
| Nitrogen bases    | do      | 16.4 |
| First acidaffins  | do      | 36.0 |
| Second acidaffins | do      | 39.8 |
| Paraffins         | do      | 7.8  |
| $N+A_1/P+A_2$     |         | 1.1  |

The reclaimed asphalt has the following composition:

|                   | Percent   |
|-------------------|-----------|
| 25 Asphaltenes    | 36.2      |
| Maltenes:         |           |
| Nitrogen bases    | 9.0       |
| First acidaffins  | 10.5      |
| Second acidaffins | 35.8      |
| 30                | 55.3 55.3 |
| Paraffins         | 8.5       |
| $N+A_1/P+A_2$     | 100.0     |
| 35                | .44       |

Thus, adding maltenes of ratio in excess of 0.4, to wit, of ratio 1.1, the deteriorated weathered asphalt of ratio 0.35 was raised to approximately the ratio of the original asphalt.

I may thus, by adding maltenes of ratio in the range of 0.4 and higher, in amounts equal to the difference between the asphaltenes content of the weathered asphalt and the asphaltenes content of the original asphalt, obtain a reclaiming of the weathered asphalt.

#### EXAMPLE 7

The surface of a three-year-old plant-mixed, hot-laid asphaltic pavement, two inches thick, used as a taxiway for aircraft, had become very brittle and porous. An attempt was made to protect the pavement from further deterioration by the application of an asphalt emulsion at a rate of approximately 0.05 gallon per square yard (a practice commonly referred to in the paving industry as "black-sealing" or "fog-sealing"). Within a few months the "sealed" surface had again become "dry" and porous. A part of the pavement was reclaimed by a sprayed-on application at the rate of 0.15 gallon per square yard of an emulsion containing:

|                                                                                                 |         |       |
|-------------------------------------------------------------------------------------------------|---------|-------|
| 60 Cationic emulsifier (fatty amido-amino amine propionate) Promeeen 2115, Process Chemical Co. | percent | 0.75  |
| Nonionic emulsifier (dodecyl phenol polyethoxy ethanol) Pronon 280, Process Chemical Co.        | do      | 0.72  |
| Water                                                                                           | do      | 50.56 |
| 65 Maltenes of the following composition:                                                       | do      | 48.00 |
| Nitrogen bases                                                                                  | do      | 12    |
| First acidaffins                                                                                | do      | 18    |
| Second acidaffins                                                                               | do      | 44    |
| Paraffins                                                                                       | do      | 26    |
| $N+A_1/P+A_2$                                                                                   |         | 43    |

After application of the emulsion, the pavement appeared fresh and "live," and no longer showed porosity or cracks. During the subsequent winter and rainy season, adjacent, un-reclaimed sections of the pavement de-

veloped large longitudinal cracks, with loosening of aggregate. The reclaimed sections showed no signs of distress.

## EXAMPLE 8

An abandoned road, consisting of a cracked and brittle asphaltic pavement of unknown history varying in thickness from three inches to about five inches, and averaging about four inches, was reclaimed by a sprayed-on application at the rate of 0.3 gallon per square yard of an emulsion substantially identical with that described in Example 7, except for the composition of the maltenes, which was:

|                   |         |     |
|-------------------|---------|-----|
| Nitrogen bases    | percent | 8   |
| First acidaffins  | do      | 14  |
| Second acidaffins | do      | 20  |
| Paraffins         | do      | 58  |
| $N+A_1/P+A_2$     |         | 282 |

At the time of the reclaiming operation, some portions of the pavement had been broken into pieces about one to two square feet in area, due to the passage of heavy tracked vehicles across the pavement; the remainder was substantially undisturbed, with random-spaced cracks typical of a weathered road surface. The reclaiming agent softened the hard and brittle asphaltic binder of the abandoned road sufficiently that it became usable in the same manner as a new paving mixture. See the following Table XIV for asphalt composition.

TABLE XIV

Composition of the Asphaltic Binder in Example 8

|                             | Composition (percent) |                   |
|-----------------------------|-----------------------|-------------------|
|                             | Before re-claiming    | After re-claiming |
| Asphaltenes                 | 26                    | 23                |
| Nitrogen bases              | 33                    | 30                |
| First acidaffins            | 8                     | 9                 |
| Second acidaffins           | 19                    | 19                |
| Paraffins                   | 14                    | 19                |
| $N+A_1/P+A_2$               | 1.24                  | 1.0               |
| Percent Asphalt in pavement | 4.41                  | 5.04              |

In the above treatment of weathered asphalt pavements, it has been found to be of considerable value to incorporate into the above emulsion employed in treating the structure a coloring agent to impart a distinctive color. A pink colored emulsion has been found effective. The structure, wetted by the emulsion, will appear colored pink. As the emulsion penetrates, the color gradually disappears. The rate of disappearance of the color serves as an indicator of the rate of penetration of the oil phase of the emulsion into the structure and guides the applicator in applying the emulsion. It permits the control of the rate of application, i.e., the gallons of emulsion spread per square yard of the road, where the road is the structure treated.

It has been found that, in order to have a colored emulsion suitable for the above purpose, it is not sufficient to employ a water-soluble dye. The dye must be an oil-soluble dye, such as has been used in dyeing of gasolines and other petroleum products. Any dye which will give a distinctive color to the emulsion when spread on the road may be employed. A red dye is suitably employed and produces a pink emulsion. Such dyes are well known in the art.

An example of a red dye suitable for this purpose is Petrol Red AB-4, sold by Patent Chemicals, Incorporated, Paterson, New Jersey. Other dyes which may be used are "Ethyl" Oil Soluble Dye—Red 100, described as follows: Azobenzene-4-azo-2-naphthol (methyl derivatives), listed as: Colour Index No. 248 (methyl derivatives); Colour Index (2nd Edition) Solvent Red 23 (methyl derivatives), No. 26100 (methyl derivatives). See Specifi-

cations ASTM D 910-57T and MIL-G-5572 B for red dye to be used in commercial and military aviation gasolines.

The dye must be first dissolved in the oil phase before emulsification, to serve as the indicator in the above application. The amount of dye to be used should be sufficient to impart a distinctive color to the emulsion. For example, an amount of the above dyes less than 1%, for example 0.03% to 1% of the oil phase of the cationic-nonionic emulsions described above has been found adequate for the above purpose.

While I have described particular embodiments of my invention, it should be understood that various modifications and adaptations thereof may be made within the spirit of the invention, as set forth in the appended claims.

I claim:

1. A method of treating asphalt containing asphaltenes, and components chosen from the group consisting of nitrogen bases, first acidaffins, second acidaffins and paraffins, said asphalts having a ratio  $N+A_1/P+A_2$  equal to  $R_a$ , where  $N$ ,  $A_1$ ,  $A_2$  and  $P$  are respectively the weight percent of the nitrogen bases, first acidaffins, second acidaffins, and paraffins present in said asphalt to be treated, which comprises treating said asphalt with an aqueous emulsion of an oil being substantially free of fractions boiling below about 160° C. at 10 millimeters of mercury absolute pressure substantially free of asphaltenes and containing components chosen from the group consisting of nitrogen bases, first acidaffins and second acidaffins and paraffins and having ratio  $R_0$  equal to about from 0.01 to less than about 19, where  $R_0$  is equal to  $N'+A'_1/P'+A'_2$  where  $N'$ ,  $A'_1$ ,  $A'_2$  and  $P'$  are respectively the weight percent of the nitrogen bases, first acidaffins, second acidaffins and paraffins present in said petroleum oil, said asphalt and said oil being employed in the ratio (Z) of the weight of oil to the weight of asphalt to form a treated asphalt of ratio  $R$  equal to

$$N''+A''_1/P''+A''_2$$

40 where  $N''$ ,  $A''_1$ ,  $A''_2$  and  $P''$  are each respectively the weight percent of the nitrogen bases, first acidaffins, second acidaffins and paraffins in said treated asphalt where  $P''$  is less than about 40%, said asphalt of ratio  $R_a$  and said oil being employed in the ratio Z, where

$$Z = \frac{(P+A_2)(R_a-R)}{(P'+A'_2)(R-R_0)}$$

where  $R$  is a value in the range from about 0.4 to about 10; and where  $R_a$  is less than 0.4,  $R$  is larger than  $R_a$ ; and where  $R_a$  is more than about 10,  $R$  is less than about 10 and less than  $R_a$ .

2. The process of claim 1, in which the oil has an initial boiling point at 10 millimeters mercury absolute pressure of above about 160° C., and is substantially free of fractions boiling below about 200° C.

3. The process of claim 1, in which  $P'$  is from about 5% to about 95% and the value of  $Z$  is not greater than that sufficient to produce an asphalt of penetration of not more than about 300.

4. The process of claim 3, in which the oil has an initial boiling point at 10 millimeters mercury absolute pressure of above about 160° C., and is substantially free of fractions boiling below about 200° C.

5. The process of claim 1, in which  $R$  has a value in the range of about 0.4 to about 1.5.

6. The process of claim 5, in which the oil has an initial boiling point at 10 millimeters mercury absolute pressure of above about 160° C., and is substantially free of fractions boiling below about 200° C.

7. The process of claim 5, in which  $P'$  is from about 5% to about 95% and the value of  $Z$  is not greater than that sufficient to produce an asphalt having a penetration of not more than about 300.

8. The process of claim 7, in which the oil has an initial boiling point at 10 millimeters mercury absolute

pressure of above about 160° C., and is substantially free of fractions boiling below about 200° C.

9. A method of treating weathered asphalt pavements formed of asphalt and aggregate, which comprises contacting the asphalt phase in said asphaltic pavements with an aqueous emulsion of petroleum oil having an initial boiling point at 10 millimeters mercury absolute pressure of above about 160° C., said oil containing components chosen from the group consisting of the nitrogen bases, first acidaffins, second acidaffins, paraffins, said oil having a ratio  $R_0$  equal to  $N' + A'_1/P' + A'_2$ , where  $N'$ ,  $A'_1$ ,  $A'_2$  and  $P'$  are each respectively the percent by weight of nitrogen bases, first acidaffins, second acidaffins and paraffins present in said oil, said asphalt of said asphalt phase having a ratio  $R_a$  equal to  $N + A_1/P + A_2$ , where  $N$ ,  $A_1$ ,  $A_2$  and  $P$  are respectively the weight percent of the nitrogen bases, first acidaffins, second acidaffins and paraffins present in said weathered asphalt, said asphalt being chosen from the group of asphalts consisting of asphalts having an  $R_a$  less than 0.4 and asphalts having an  $R_a$  more than 1.5, thereby adjusting the ratio  $R_a$  of said asphalt to a ratio  $R$  equal to  $N'' + A''_1/P'' + A''_2$ , where  $N''$ ,  $A''_1$ , and  $A''_2$ , and  $P''$  are respectively the weight percent of the nitrogen bases, first acidaffins, second acidaffins and paraffins present in the reclaimed asphalt phase of said asphaltic pavement, and where  $P''$  is less than about 40%, the value of said ratio  $R_0$  being greater than the value of said ratio  $R_a$  when  $R_a$  is less than 0.4, and said ratio  $R_0$  being less than  $R_a$  when said ratio  $R_a$  is greater than 1.5.

10. The process of claim 9, in which said emulsion contains an emulsifier chosen from the group consisting of the anionic, cationic and nonionic emulsifiers and a mixture of cationic and nonionic emulsifiers.

11. The process of claim 10, in which the emulsion is a cationic emulsion and contains cationic emulsifiers from about 0.5% to 1.2% of the weight of the oil phase in said emulsion and nonionic emulsifier from about 0.5% to 2% by weight of said oil phase.

12. A method of treating asphalt pavement, the asphalt of said pavement containing components chosen from the group consisting of asphaltenes, nitrogen bases, first acidaffins, paraffins, and second acidaffins, said method comprising applying to said pavement an emulsion of a petroleum oil, substantially free of asphaltenes and consisting essentially of components chosen from the group consisting of nitrogen bases ( $N'$ ), first acidaffins ( $A'_1$ ), paraffins ( $P'$ ), and second acidaffins ( $A'_2$ ), where  $N'$ ,  $A'_1$ ,  $P'$ ,  $A'_2$  are respectively the weight percent of the nitrogen bases, first acidaffins, paraffins and second acidaffins, in the said petroleum oil, and said components being in the ratio of  $N' + A'_1/P' + A'_2$  equaling a value of from about 0.01 to about 19, said oil having an initial boiling point at 10 millimeters of mercury absolute pressure of over 160° C., said emulsion containing an emulsifier, the petroleum oil of said emulsion combining with said asphalt of said pavement, producing a treated asphalt containing components chosen from the group consisting of nitrogen bases, first acidaffins, paraffins and second acidaffins, said components being in the ratio  $N'' + A''_1/P'' + A''_2$  where  $N''$ ,  $A''_1$ ,  $P''$ ,  $A''_2$  are respectively the weight percent of the nitrogen bases, first acidaffins, paraffins and second acidaffins in the asphalt containing said petroleum oil, said last named ratio equaling a value of from about 0.4 to less than about 10, and said  $P''$  being not more than 40%, said asphalt containing said oil having a penetration within the 200-300 penetration grade.

13. In the method of claim 12, said oil being substantially free of fractions boiling below about 200° C. at said pressure.

14. In the process of claim 12, the amount of the oil incorporated in said asphalt phase in the upper section of said asphaltic road pavement being sufficient to adjust the ratio  $N'' + A''_1/P'' + A''_2$  in said asphalt phase of said asphaltic pavement to the range of about 0.4 to about 1.5

in the reclaimed asphalt phase of said top section of said road, the amount of oil added increasing the asphalt content of said asphaltic concrete pavement to not in excess of about 8% of the weight of the asphalt plus the aggregate in said section.

15. A method for reclaiming weathered asphalt which comprises commingling asphalt with an aqueous emulsion of a petroleum oil being substantially free of fractions boiling below about 160° C. at 10 millimeters of mercury absolute pressure substantially free of asphaltenes and containing paraffins components in about 5% to about 95% by weight of said oil and containing also components selected from the group consisting of the nitrogen bases, first acidaffins and second acidaffins, said components being present in concentration in said oil such that the ratio  $N' + A'_1/P' + A'_2$  is equal to from about 0.01 to about 19, where  $N'$ ,  $A'_1$ ,  $A'_2$  and  $P'$  are respectively the weight percent of the nitrogen bases, first acidaffins, second acidaffins and paraffins present in said oil, and thereby producing a reclaimed asphalt having a ratio  $N'' + A''_1/P'' + A''_2$  of from about 0.4 to about 1.5, where  $N''$ ,  $A''_1$ ,  $A''_2$  and  $P''$  are respectively the weight percent of the nitrogen bases, first acidaffins and second acidaffins and paraffins present in said reclaimed asphalt, and  $P''$  is less than about 40%, said emulsion containing an emulsifier.

16. The method of claim 15, said aqueous emulsion containing an emulsifier chosen from the group consisting of the anionic, cationic, nonionic, and mixed cationic and nonionic emulsifiers.

17. The process of claim 16, in which the emulsion is a cationic emulsion containing cationic and nonionic emulsifiers, said cationic emulsifier being in the range of about 0.5% to about 1.2% by weight of the oil phase in said emulsion and said nonionic emulsifier being in the range of about 0.5% to about 2% of the weight of said oil phase.

18. A method of reclaiming weathered asphalt pavement comprising applying to the surface of said weathered pavement a cationic emulsion of petroleum oil having an initial boiling point at 10 millimeters mercury pressure absolute above about 160° C., and being substantially free of asphaltenes, and containing components chosen from the group consisting of the nitrogen bases, first acidaffins, second acidaffins and paraffins, the ratio  $N' + A'_1/P' + A'_2$  being in the range of about 0.01 to about 19, where  $N'$ ,  $A'_1$ ,  $A'_2$  and  $P'$  are respectively the weight percent of the nitrogen bases, first acidaffins, second acidaffins and paraffins present in said oil, said emulsion being added in amounts sufficient to increase asphaltic content in said asphaltic pavement to a percent not greater than about 8% of said asphaltic pavement in the top section of said pavement to adjust the ratio  $N'' + A''_1/P'' + A''_2$  in said asphalt phase in said section to more than about 0.4 and less than about 1.5, where  $N''$ ,  $A''_1$ ,  $A''_2$  and  $P''$  are the percent by weight of the nitrogen bases, first acidaffins, second acidaffins and paraffins present in said reclaimed asphalt phase in said section and  $P''$  is less than about 40%.

19. The process of claim 18, in which the cationic emulsion contains from about 0.5% to about 1.2% by weight of a cationic emulsifier and from 0.5% to about 2% by weight of a nonionic emulsifier, based on the oil phase of said emulsion.

20. The process of claim 18, applying said oil in said emulsion containing about 40% of oil phase in quantities per square yard equivalent to that at least in amounts per square yard sufficient to be absorbed in the weathered pavement within the first fifteen minutes upon gradual application of said emulsion to said pavement.

21. The process of claim 20, in which the cationic emulsion contains from about 0.5% to about 1.2% by weight of a cationic emulsifier and from 0.5% to about 2% by weight of a nonionic emulsifier, based on the oil phase of said emulsion.

22. A method of reclaiming a weathered asphalt pavement, the asphalt phase of said pavement containing asphaltenes, nitrogen bases, first acidaffins, second acidaffins

and paraffins and having a ratio  $N+A_1/P+A_2$  equal to  $R_a$ , where  $N$ ,  $A_1$ ,  $A_2$  and  $P$  are respectively the weight percent of the nitrogen bases, first acidaffins, second acidaffins and paraffin components, respectively, present in said asphalt phase, said weathered asphalt being chosen from the group consisting of asphalts having  $R_a$  less than 0.4 and asphalts having a ratio  $R_a$  larger than 1.5, which comprises treating said asphalt with an aqueous emulsion of a petroleum oil substantially free of asphaltenes, having ratio  $R_0$  equal to about 0.4, where  $R_0$  is equal to  $N'+A'_1/P'+A'_2$ , where  $N'$ ,  $A'_1$ ,  $A'_2$  and  $P'$  are respectively the weight percent of the nitrogen bases, first acidaffins, second acidaffins and paraffins present in said petroleum oil, said oil having an initial boiling point above about 160° C. at 10 mm. mercury absolute pressure, said emulsion containing an emulsifier, said asphalt and said oil being employed in the ratio of the weight of oil to the weight of asphalt to form a reclaimed asphalt phase in said pavement having a ratio  $R$ , where  $R$  is equal to  $N''+A''_1/P''+A''_2$ , where  $N''$ ,  $A''_1$ ,  $A''_2$  and  $P''$  are each respectively the weight percent of the nitrogen bases, first acidaffins, second acidaffins and paraffins present in said reclaimed asphalt phase, and thereby adjusting the ratio  $R$  in the direction of the range of above about 0.4, said reclaimed asphalt having a ratio  $R$  in excess of 0.4.

23. The process of claim 22, in which  $R$  has a value in the range of about 0.4 to about 1.5.

24. The method of claim 22, said aqueous emulsion containing an emulsifier chosen from the group consisting of the cationic, nonionic and mixed cationic and non-ionic emulsifiers.

25. The process of claim 24, in which the emulsion is a cationic emulsion containing cationic and nonionic emulsifiers, said cationic emulsifier being in the range of about 0.5% to about 1.2% by weight of the oil phase in said emulsion and said nonionic emulsifier being in the range of about .5% to about 2% of the weight of said oil phase.

26. A method for reclaiming weathered asphalt containing asphaltenes, nitrogen bases, first acidaffins and second acidaffins, which comprises commingling with said asphalt an aqueous cationic emulsion of a petroleum fraction substantially free of asphaltenes, and containing paraffins in the range of about 20% to about 85% by weight of said petroleum fractions, the remaining portion of said petroleum fraction being nitrogen bases, first acidaffins and second acidaffins.

27. In the process of claim 26, adding said petroleum fraction to said asphalt in an amount sufficient in quantity to penetrate into and become incorporated in the asphalt, but insufficient to produce a free oil phase, said aqueous medium containing a nonionic surfactant and a cationic surfactant, said nonionic surfactant being in the range of about 0.5% to about 2.0% of said oil phase, and said cationic surfactant being in the range of about 0.5% to 1.5% by weight of said oil phase, said water content being not less than about 25% by weight of said emulsion.

28. In the method of claim 26, said nitrogen bases in said petroleum fraction being in an amount not more than 20% by weight of said petroleum fraction, and said first acidaffins being in an amount not more than about 20% by weight of said petroleum fraction, and paraffins and second acidaffins in an amount sufficient to equal to 100% by weight when added to the percent by weight of said nitrogen bases, first acidaffins and paraffins.

29. The process of claim 26, said petroleum fraction containing not more than about 35% by weight of a mixture of nitrogen bases and first acidaffins, the remaining portion of said petroleum fraction being composed of paraffins and second acidaffins.

30. A method of reclaiming weathered asphalt pavement containing asphaltenes, nitrogen bases, first acidaffins and second acidaffins, which comprises comminuting the asphalt pavement by scarifying the same and discing the scarified pavement, spraying the comminuted road

surface with a cationic emulsion in an amount in the range of about one-fourth to one-half gallon of emulsion per square yard of said broken, comminuted road surface per inch of depth, said emulsion comprising an aqueous phase and a cationic surfactant, and a petroleum fraction dispersed therein as a positively charged dispersed oil phase, said petroleum fraction substantially free of asphaltenes, and containing paraffins in the range of about 20% to about 85% by weight of said petroleum fraction, and the remaining portion of said petroleum fraction being composed of nitrogen bases, first acidaffins and second acidaffins.

31. A process for reclaiming weathered asphaltic pavement composed of weathered asphalt and aggregate, said weathered asphalt containing asphaltenes, nitrogen bases, first acidaffins and second acidaffins, which comprises applying to said weathered asphalt pavement a cationic emulsion of a petroleum fraction, said fraction substantially free of asphaltenes and containing paraffins in the

range of about 20% to about 85% by weight of said petroleum fraction, the remaining portion of said petroleum fraction being composed of nitrogen bases, first acidaffins and second acidaffins, adding said petroleum fraction to said asphalt in an amount sufficient in quantity to penetrate into and become incorporated in the asphalt, but insufficient to produce a free oil phase, said emulsion containing a nonionic surfactant and a cationic surfactant, said nonionic surfactant being in the range of about 0.5% to about 2.0% of said oil phase, and said cationic surfactant being in the range of about 0.5% to 1.5% by weight of said oil phase, said water content being not less than about 25% by weight of said emulsion.

32. A method of maintaining the resistance of asphaltic pavements to weathering, which asphalt pavement contains asphalt comprising asphaltenes and containing nitrogen bases, first acidaffins, second acidaffins and paraffins, which comprises spreading upon said pavement, at a time not later than the first development of hair cracks in said pavement by weathering, a cationic aqueous oil emulsion in the amount of from 0.05 to 0.15 gallon per square yard per inch of depth of said asphaltic pavement, and a petroleum fraction dispersed therein, said petroleum fraction substantially free of asphaltenes, and containing paraffins in the range of about 20% to about 85% by weight of said petroleum fraction, and the remaining portion of said petroleum fraction being composed of nitrogen bases, first acidaffins and second acidaffins.

33. In the method of claim 32, the nitrogen bases in said petroleum fraction being not more than about 35% by weight of a mixture of nitrogen bases and first acidaffins, the remaining portion of said petroleum fraction being composed of paraffins and second acidaffins, said paraffins being in the range of about 20% to about 85% of said petroleum fraction.

34. A method of reclaiming an asphalt composition of aggregate bonded by weathered asphalt, containing asphaltenes, nitrogen bases, first acidaffins and second acidaffins, said weathered asphalt containing less than about 10% of paraffins, to produce an asphalt composition in which said aggregate is bonded by reclaimed asphalt, which comprises applying to said weathered asphaltic composition, a cationic emulsion of a petroleum fraction substantially free of asphaltenes, containing paraffins in the range of about 20% to about 85% of said petroleum fraction, the remaining portion of said petroleum fraction being composed of nitrogen bases, first acidaffins and second acidaffins, said emulsion being added in amounts sufficient to increase the asphaltic content of said asphaltic composition and to increase the paraffins content of said reclaimed asphalt to substantially above 10%.

35. A method of reclaiming a weathered asphalt pavement originally of a composition comprising aggregate and asphalt of specification grade of penetration and in specification amounts in said pavement, and which, on weathering, produces a weathered pavement, including a

weathered asphalt containing asphaltenes, nitrogen bases, first acidaffins and second acidaffins, and having less than about 10% of paraffins, which method comprises applying to said weathered pavement a cationic water emulsion of a petroleum fraction substantially free of asphaltenes, containing paraffins in the range of about 20% to 85% of said petroleum fraction, and the remaining portion of said petroleum fraction being composed of nitrogen bases, first acidaffins and second acidaffins, said emulsion being applied in an amount sufficient to increase the asphaltic content of said asphaltic aggregate composition from about 1.2 to about 1.3 times that of said specification amounts of said asphalt in said original composition of said pavement and adding to said weathered asphalt paraffins to produce a reclaimed asphalt containing an amount of paraffins substantially above 10% and to produce a reclaimed asphalt having a penetration value substantially higher than the penetration value of said weathered asphalt, but within said penetration range of 30-300.

36. A method of reclaiming weathered asphalt pavement composed of aggregate and weathered asphalt, which weathered asphalt contains asphaltenes, nitrogen bases, first acidaffins and second acidaffins, and has less than about 10% of paraffins, which comprises applying to said pavement an aqueous cationic emulsion of a petroleum fraction substantially free of asphaltenes containing paraffins in the range of about 20% to about 85% of said petroleum fraction, the remaining portion of said petroleum fraction being composed of nitrogen bases, first acidaffins and second acidaffins, said petroleum fractions being added in amount sufficient to produce reclaimed asphalt pavement containing reclaimed asphalt in amounts substantially above the asphaltic content of said weathered asphalt pavement, and to substantially increase the paraffins content of said reclaimed asphalt to above 10%.

37. A method of repairing weathered asphalt pavements containing asphaltenes, nitrogen bases, first acidaffins and second acidaffins, which comprises spraying on said pavement an aqueous cationic emulsion containing as the dispersed phase a petroleum fraction substantially free of asphaltenes and containing paraffins from about 20% to about 85% by weight of said petroleum fractions and the remaining portion of said petroleum fractions being composed of nitrogen bases, first acidaffins and second acidaffins, in amounts sufficient to produce a reclaimed asphalt substantially free of syneresis of said oil phase from said reclaimed asphalt pavement.

38. The process of claim 37, in which said emulsion is spread in amounts within the range of above about 0.05 of a gallon of emulsion per square yard per inch of depth of said pavement and in amounts sufficient to give an asphalt in said repaired asphalt pavement containing more than about 10% of paraffins.

39. A method of reclaiming weathered asphaltic pavement composition comprising aggregate and weathered asphalt, said weathered asphalt containing asphaltenes and which pavement was originally formed with asphalt fractions of not more than 6% by weight of the asphalt-aggregate composition, the asphaltenes in said weathered asphalt consisting of the asphaltenes originally present in the asphalt fraction and asphaltenes formed by weathering, the amount of said weathered asphalt in said pavement composition, calculated by excluding from said weathered asphalt the amount of the asphaltenes content formed by said weathering, being in amounts less than the asphalt content in the original asphaltic pavement composition, and said weathered asphalt containing also nitrogen bases, first acidaffins and second acidaffins, and having less than about 10% of paraffins, which method comprises applying to said pavement composition at cationic water emulsion of a petroleum fraction substantially free of asphaltenes and containing paraffins in the range of about 20% to 85% of said petroleum fraction, the remaining portion of said petroleum fraction being com-

posed of nitrogen bases, first acidaffins and second acidaffins, said petroleum fraction being added in amounts sufficient to increase the asphaltic content of the asphaltic pavement substantially above the asphaltic content of the weathered pavement and up to about 1.3 times the asphaltic content of the asphalt-aggregate composition as originally formed and prior to weathering, to produce a reclaimed asphalt in said asphalt-aggregate mix containing substantially more than 10% of paraffins.

10 40. A method of treating weathered asphalt containing asphaltenes, nitrogen bases, first acidaffins and second acidaffins, which comprises mixing with said weathered asphalt an aqueous emulsion of a petroleum oil fraction substantially free of asphaltenes, containing from about 15 20% to about 85% by weight of paraffins, the remaining portion of the petroleum oil fraction containing nitrogen bases, first acidaffins and second acidaffins, said oil having an initial boiling point at 10 millimeters mercury absolute pressure of above about 160° C., and said emulsion containing a surface active agent.

20 41. The process of claim 40, said surface active agent containing a nonionic and a cationic surfactant, said non-ionic surfactant being in the range of about 0.5% to about 2.0% of said oil phase, and said cationic surfactant being 25 in the range of about 0.5% to 1.5% by weight of said oil phase, said water content being not less than about 25% by weight of said emulsion.

30 42. The process of treating a weathered asphalt pavement composed of aggregate and weathered asphalt, said weathered asphalt containing asphaltenes, nitrogen bases, first acidaffins and second acidaffins, which comprises spreading on said road an aqueous emulsion of a petroleum oil fraction substantially free of asphaltenes, containing from about 20% to about 85% by weight of paraffins, the remaining portion of the petroleum oil fraction containing nitrogen bases, first acidaffins and second acidaffins, said oil having an initial boiling point at 10 millimeters mercury absolute pressure of above about 160° C., and said emulsion containing a surface 35 active agent.

40 43. The process of claim 42, said emulsion containing a nonionic surfactant and a cationic surfactant, said non-ionic surfactant being in the range of about 0.5% to about 2.0% of said oil phase, and said cationic surfactant being 45 in the range of about 0.5% to 1.5% by weight of said oil phase, said water content being not less than about 25% by weight of said emulsion.

44. A process for reclaiming weathered asphaltic pavement composed of weathered asphalt and aggregate, which comprises applying to the weathered asphalt an amount of an emulsion containing a petroleum oil substantially free of asphaltenes, and containing resinous oil components in an amount of at least 15% of the said resinous 50 petroleum oil, the remaining being substantially paraffins sufficient to form an amount of reclaimed asphalt equal to at least 4% and not more than 8% of the weight of the aggregate plus the reclaimed asphalt, the amount of said petroleum oil component of said emulsion added 55 being in amount such that a sample of said reclaimed weathered asphalt pavement, when extracted to separate the extract asphalt from said aggregate, and analyzing the extract asphalt to determine the asphaltene content and the resin content and the paraffins of said extract asphalt, and making a sieve analysis of said aggregate to determine the rock portion thereof retained on a four-mesh screen, the sand portion thereof passing through a four-mesh screen and retained on a 200-mesh screen, and the silt portion thereof passing a 200-mesh screen, the amount of said 60 resinous oil added is in an amount sufficient such that the sum of the resinous components and paraffins of said petroleum oil added to said weathered asphalt results in extract asphalt which is equal to a percentage of the total mixture of reclaimed asphalt and aggregate equal to from 65 70 75

about  $P$  to  $1.3 \times P$ , where  $P$  is determined by the following formula:

$$P = (R \times 4 + S \times 7 + F \times 12)$$

where  $R$  is the decimal percentage of the rock portion of said aggregate,  $S$  is the decimal percentage of the sand portion of said aggregate, and  $F$  is the decimal percentage of the silt portion of said aggregate.

45. In the process of claim 44, said emulsion containing a nonionic and a cationic surfactant, said nonionic surfactant being in the range of about 0.5% to about 2.0% of said oil phase, and said cationic surfactant being in the range of about 0.5% to 1.5% by weight of said oil phase, said water content being not less than about 25% by weight of said emulsion.

46. A method of treating asphalt pavement, the asphalt of said pavement containing components chosen from the group consisting of asphaltenes, nitrogen bases, first acidaffins, paraffins, and second acidaffins, said method comprising applying to said pavement an emulsion of a petroleum oil, substantially free of asphaltenes and consisting essentially of components chosen from the group consisting of nitrogen bases ( $N'$ ), first acidaffins ( $A_1'$ ), paraffins ( $P'$ ), and second acidaffins ( $A_2'$ ), where  $N'$ ,  $A_1'$ ,  $P'$ ,  $A_2'$  are respectively the weight percent of the nitrogen bases, first acidaffins, paraffins and second acidaffins, in the said petroleum oil, and said components being in the ratio of  $N' + A_1' / P' + A_2'$  equaling a value of from about 0.01 to about 19, said oil having an initial boiling point

at 10 millimeters of mercury absolute pressure of over 160° C., said emulsion containing an emulsifier, the petroleum oil of said emulsion combining with said asphalt of said pavement, producing a treated asphalt containing 5 components chosen from the group consisting of nitrogen bases, first acidaffins, paraffins and second acidaffins, said components being in the ratio  $N'' + A_1'' / P'' + A_2''$  where  $N''$ ,  $A_1''$ ,  $P''$ ,  $A_2''$  are respectively the weight percent of the nitrogen bases, first acidaffins, paraffins and second acidaffins in the asphalt containing said petroleum oil, 10 said ratio equaling a value of from about 0.4 to about 1.5, and said  $P''$  being not more than 40%.

47. In the method of claim 46, said oil being substantially free of fractions boiling below about 200° C. at said 15 pressure.

References Cited by the Examiner

UNITED STATES PATENTS

|           |       |             |       |          |
|-----------|-------|-------------|-------|----------|
| 1,926,523 | 9/33  | Fulton      | ----- | 260—28.5 |
| 2,131,205 | 9/38  | Wells       | ----- | 94—23 X  |
| 2,639,651 | 5/53  | Scott       | ----- | 94—23    |
| 2,701,213 | 2/55  | Neville     | ----- | 94—23    |
| 2,706,688 | 4/55  | Sommer      | ----- | 106—277  |
| 2,728,684 | 12/55 | Darragh     | ----- | 106—285  |
| 2,876,686 | 3/59  | Birney      | ----- | 94—23    |
| 2,928,752 | 3/60  | Felletschin | ----- | 106—285  |

JACOB L. NACKENOFF, Primary Examiner.

HENRY C. SUTHERLAND, Examiner.